



US009057242B2

(12) **United States Patent**  
**Mazyar et al.**

(10) **Patent No.:** **US 9,057,242 B2**  
(45) **Date of Patent:** **Jun. 16, 2015**

(54) **METHOD OF CONTROLLING CORROSION RATE IN DOWNHOLE ARTICLE, AND DOWNHOLE ARTICLE HAVING CONTROLLED CORROSION RATE**

(75) Inventors: **Oleg A. Mazyar**, Houston, TX (US); **Michael Johnson**, Katy, TX (US); **Sean Gaudette**, Katy, TX (US)

(73) Assignee: **Baker Hughes Incorporated**, Houston, TX (US)

(\*) Notice: Subject to any disclaimer, the term of this patent is extended or adjusted under 35 U.S.C. 154(b) by 861 days.

(21) Appl. No.: **13/204,359**

(22) Filed: **Aug. 5, 2011**

(65) **Prior Publication Data**

US 2013/0032357 A1 Feb. 7, 2013

(51) **Int. Cl.**

**E21B 29/00** (2006.01)  
**E21B 34/06** (2006.01)  
**E21B 34/14** (2006.01)  
**E21B 33/12** (2006.01)  
**E21B 41/00** (2006.01)

(52) **U.S. Cl.**

CPC ..... **E21B 34/063** (2013.01); **E21B 34/14** (2013.01); **E21B 33/12** (2013.01); **E21B 29/00** (2013.01); **E21B 41/00** (2013.01)

(58) **Field of Classification Search**

CPC ..... E21B 10/00; E21B 44/00; E21B 33/12; E21B 43/26; E21B 17/028; E21B 23/00

USPC ..... 166/376  
See application file for complete search history.

(56)

**References Cited**

U.S. PATENT DOCUMENTS

|             |         |                   |
|-------------|---------|-------------------|
| 1,468,905 A | 9/1923  | Herman            |
| 2,238,895 A | 4/1941  | Gage              |
| 2,261,292 A | 11/1941 | Salnikov          |
| 2,294,648 A | 9/1942  | Ansel et al.      |
| 2,301,624 A | 11/1942 | Holt              |
| 2,754,910 A | 7/1956  | Derrick et al.    |
| 2,983,634 A | 5/1961  | Budininkas et al. |
| 3,057,405 A | 10/1962 | Mallinger         |
| 3,106,959 A | 10/1963 | Huitt et al.      |
| 3,152,009 A | 10/1964 | DeLong            |
| 3,196,949 A | 7/1965  | Thomas            |
| 3,242,988 A | 3/1966  | McGuire et al.    |

(Continued)

FOREIGN PATENT DOCUMENTS

|    |           |         |
|----|-----------|---------|
| CN | 1076968   | 10/1993 |
| CN | 1255879 A | 11/2000 |

(Continued)

OTHER PUBLICATIONS

Canadian Pat. App. No. 2783241 filed on Dec. 7, 2010 titled Nanomatrix Powder Metal Compact.

(Continued)

*Primary Examiner* — Jennifer H Gay

*Assistant Examiner* — Caroline Butcher

(74) *Attorney, Agent, or Firm* — Cantor Colburn LLP

(57) **ABSTRACT**

A method of removing a downhole assembly comprises contacting, in the presence of an electrolyte, a first article comprising a first material and acting as an anode, and a second article comprising a second material having a lower reactivity than the first material and acting as a cathode, the downhole assembly comprising the first article in electrical contact with the second article, wherein at least a portion of the first article is corroded in the electrolyte.

**21 Claims, 4 Drawing Sheets**



| (56)                  | References Cited |                       |             |         |                    |
|-----------------------|------------------|-----------------------|-------------|---------|--------------------|
| U.S. PATENT DOCUMENTS |                  |                       |             |         |                    |
| 3,316,748 A           | 5/1967           | Lang et al.           | 4,949,788 A | 8/1990  | Szarka et al.      |
| 3,347,317 A           | 10/1967          | Zandemer              | 4,952,902 A | 8/1990  | Kawaguchi et al.   |
| 3,347,714 A           | 10/1967          | Broverman et al.      | 4,975,412 A | 12/1990 | Okazaki et al.     |
| 3,390,724 A           | 7/1968           | Caldwell              | 4,977,958 A | 12/1990 | Miller             |
| 3,395,758 A           | 8/1968           | Kelly et al.          | 4,981,177 A | 1/1991  | Carmody et al.     |
| 3,406,101 A           | 10/1968          | Kilpatrick            | 4,986,361 A | 1/1991  | Mueller et al.     |
| 3,434,537 A           | 3/1969           | Zandmer               | 4,997,622 A | 3/1991  | Regazzoni et al.   |
| 3,465,181 A           | 9/1969           | Colby et al.          | 5,006,044 A | 4/1991  | Walker, Sr. et al. |
| 3,513,230 A           | 5/1970           | Rhees et al.          | 5,010,955 A | 4/1991  | Springer           |
| 3,637,446 A           | 1/1972           | Elliott et al.        | 5,036,921 A | 8/1991  | Pittard et al.     |
| 3,645,331 A           | 2/1972           | Maurer et al.         | 5,048,611 A | 9/1991  | Cochran            |
| 3,765,484 A           | 10/1973          | Hamby, Jr. et al.     | 5,049,165 A | 9/1991  | Tselesin           |
| 3,768,563 A           | 10/1973          | Blount                | 5,061,323 A | 10/1991 | DeLucia            |
| 3,775,823 A           | 12/1973          | Adolph et al.         | 5,063,775 A | 11/1991 | Walker, Sr. et al. |
| 3,878,889 A           | 4/1975           | Seabourn              | 5,073,207 A | 12/1991 | Faure et al.       |
| 3,894,850 A           | 7/1975           | Kovalchuk et al.      | 5,074,361 A | 12/1991 | Brisco et al.      |
| 3,924,677 A           | 12/1975          | Prenner et al.        | 5,076,869 A | 12/1991 | Bourell et al.     |
| 4,010,583 A           | 3/1977           | Highberg              | 5,084,088 A | 1/1992  | Okazaki            |
| 4,039,717 A           | 8/1977           | Titus                 | 5,087,304 A | 2/1992  | Chang et al.       |
| 4,050,529 A           | 9/1977           | Tagirov et al.        | 5,090,480 A | 2/1992  | Pittard et al.     |
| 4,248,307 A           | 2/1981           | Silberman et al.      | 5,095,988 A | 3/1992  | Bode               |
| 4,372,384 A           | 2/1983           | Kinney                | 5,103,911 A | 4/1992  | Heijnen            |
| 4,373,584 A           | 2/1983           | Silberman et al.      | 5,117,915 A | 6/1992  | Mueller et al.     |
| 4,373,952 A           | 2/1983           | Parent                | 5,161,614 A | 11/1992 | Wu et al.          |
| 4,374,543 A           | 2/1983           | Richardson            | 5,178,216 A | 1/1993  | Giroux et al.      |
| 4,384,616 A           | 5/1983           | Dellinger             | 5,181,571 A | 1/1993  | Mueller et al.     |
| 4,395,440 A           | 7/1983           | Abe et al.            | 5,183,631 A | 2/1993  | Kugimiya et al.    |
| 4,399,871 A           | 8/1983           | Adkins et al.         | 5,188,182 A | 2/1993  | Echols, III et al. |
| 4,407,368 A           | 10/1983          | Erbstoesser           | 5,188,183 A | 2/1993  | Hopmann et al.     |
| 4,422,508 A           | 12/1983          | Rutledge, Jr. et al.  | 5,204,055 A | 4/1993  | Sachs et al.       |
| 4,452,311 A           | 6/1984           | Speegle et al.        | 5,222,867 A | 6/1993  | Walker, Sr. et al. |
| 4,475,729 A           | 10/1984          | Costigan              | 5,226,483 A | 7/1993  | Williamson, Jr.    |
| 4,498,543 A           | 2/1985           | Pye et al.            | 5,228,518 A | 7/1993  | Wilson et al.      |
| 4,499,048 A           | 2/1985           | Hanejko               | 5,234,055 A | 8/1993  | Cornette           |
| 4,499,049 A           | 2/1985           | Hanejko               | 5,253,714 A | 10/1993 | Davis et al.       |
| 4,526,840 A           | 7/1985           | Jarabek               | 5,271,468 A | 12/1993 | Streich et al.     |
| 4,534,414 A           | 8/1985           | Pringle               | 5,282,509 A | 2/1994  | Schurr, III        |
| 4,539,175 A           | 9/1985           | Lichti et al.         | 5,293,940 A | 3/1994  | Hromas et al.      |
| 4,554,986 A           | 11/1985          | Jones                 | 5,304,260 A | 4/1994  | Aikawa et al.      |
| 4,640,354 A           | 2/1987           | Boisson               | 5,309,874 A | 5/1994  | Willermet et al.   |
| 4,664,962 A           | 5/1987           | DesMarais, Jr.        | 5,310,000 A | 5/1994  | Arterbury et al.   |
| 4,668,470 A           | 5/1987           | Gilman et al.         | 5,316,598 A | 5/1994  | Chang et al.       |
| 4,673,549 A           | 6/1987           | Ecer                  | 5,318,746 A | 6/1994  | Lashmore           |
| 4,674,572 A           | 6/1987           | Gallus                | 5,380,473 A | 1/1995  | Bogue et al.       |
| 4,678,037 A           | 7/1987           | Smith                 | 5,387,380 A | 2/1995  | Cima et al.        |
| 4,681,133 A           | 7/1987           | Weston                | 5,392,860 A | 2/1995  | Ross               |
| 4,688,641 A           | 8/1987           | Knieriem              | 5,394,941 A | 3/1995  | Venditto et al.    |
| 4,693,863 A           | 9/1987           | Del Corso et al.      | 5,398,754 A | 3/1995  | Dinhoble           |
| 4,703,807 A           | 11/1987          | Weston                | 5,427,177 A | 6/1995  | Jordan, Jr. et al. |
| 4,706,753 A           | 11/1987          | Ohkochi et al.        | 5,435,392 A | 7/1995  | Kennedy            |
| 4,708,202 A           | 11/1987          | Sukup et al.          | 5,439,051 A | 8/1995  | Kennedy et al.     |
| 4,708,208 A           | 11/1987          | Halbardier            | 5,454,430 A | 10/1995 | Kennedy et al.     |
| 4,709,761 A           | 12/1987          | Setterberg, Jr.       | 5,456,317 A | 10/1995 | Hood, III et al.   |
| 4,714,116 A           | 12/1987          | Brunner               | 5,464,062 A | 11/1995 | Blizzard, Jr.      |
| 4,721,159 A           | 1/1988           | Ohkochi et al.        | 5,472,048 A | 12/1995 | Kennedy et al.     |
| 4,738,599 A           | 4/1988           | Shilling              | 5,474,131 A | 12/1995 | Jordan, Jr. et al. |
| 4,768,588 A           | 9/1988           | Kupsa                 | 5,477,923 A | 12/1995 | Jordan, Jr. et al. |
| 4,775,598 A           | 10/1988          | Jaeckel               | 5,507,439 A | 4/1996  | Story              |
| 4,784,226 A           | 11/1988          | Wyatt                 | 5,526,880 A | 6/1996  | Jordan, Jr. et al. |
| 4,805,699 A           | 2/1989           | Halbardier            | 5,526,881 A | 6/1996  | Martin et al.      |
| 4,817,725 A           | 4/1989           | Jenkins               | 5,529,746 A | 6/1996  | Knoss et al.       |
| 4,834,184 A           | 5/1989           | Streich et al.        | 5,533,573 A | 7/1996  | Jordan, Jr. et al. |
| H635 H                | 6/1989           | Johnson et al.        | 5,536,485 A | 7/1996  | Kume et al.        |
| 4,850,432 A           | 7/1989           | Porter et al.         | 5,558,153 A | 9/1996  | Holcombe et al.    |
| 4,853,056 A           | 8/1989           | Hoffman               | 5,607,017 A | 3/1997  | Owens et al.       |
| 4,869,324 A           | 9/1989           | Holder                | 5,623,993 A | 4/1997  | Van Buskirk et al. |
| 4,869,325 A           | 9/1989           | Halbardier            | 5,623,994 A | 4/1997  | Robinson           |
| 4,889,187 A           | 12/1989          | Terrell et al.        | 5,636,691 A | 6/1997  | Hendrickson et al. |
| 4,890,675 A           | 1/1990           | Dew                   | 5,641,023 A | 6/1997  | Ross et al.        |
| 4,909,320 A           | 3/1990           | Hebert et al.         | 5,647,444 A | 7/1997  | Williams           |
| 4,929,415 A           | 5/1990           | Okazaki               | 5,665,289 A | 9/1997  | Chung et al.       |
| 4,932,474 A           | 6/1990           | Schroeder, Jr. et al. | 5,677,372 A | 10/1997 | Yamamoto et al.    |
| 4,938,309 A           | 7/1990           | Emdy                  | 5,685,372 A | 11/1997 | Gano               |
| 4,938,809 A           | 7/1990           | Das et al.            | 5,701,576 A | 12/1997 | Fujita et al.      |
| 4,944,351 A           | 7/1990           | Eriksen et al.        | 5,707,214 A | 1/1998  | Schmidt            |

(56)

## References Cited

## U.S. PATENT DOCUMENTS

|              |         |                    |              |         |                      |
|--------------|---------|--------------------|--------------|---------|----------------------|
| 5,709,269 A  | 1/1998  | Head               | 6,491,116 B2 | 12/2002 | Berscheidt et al.    |
| 5,720,344 A  | 2/1998  | Newman             | 6,513,598 B2 | 2/2003  | Moore et al.         |
| 5,728,195 A  | 3/1998  | Eastman et al.     | 6,540,033 B1 | 4/2003  | Sullivan et al.      |
| 5,765,639 A  | 6/1998  | Muth               | 6,543,543 B2 | 4/2003  | Muth                 |
| 5,772,735 A  | 6/1998  | Sehgal et al.      | 6,561,275 B2 | 5/2003  | Glass et al.         |
| 5,782,305 A  | 7/1998  | Hicks              | 6,588,507 B2 | 7/2003  | Dusterhoft et al.    |
| 5,797,454 A  | 8/1998  | Hipp               | 6,591,915 B2 | 7/2003  | Burris et al.        |
| 5,826,652 A  | 10/1998 | Tapp               | 6,601,648 B2 | 8/2003  | Ebinger              |
| 5,826,661 A  | 10/1998 | Parker et al.      | 6,601,650 B2 | 8/2003  | Sundararajan         |
| 5,829,520 A  | 11/1998 | Johnson            | 6,609,569 B2 | 8/2003  | Howlett et al.       |
| 5,836,396 A  | 11/1998 | Norman             | 6,612,826 B1 | 9/2003  | Bauer et al.         |
| 5,857,521 A  | 1/1999  | Ross et al.        | 6,613,383 B1 | 9/2003  | George et al.        |
| 5,881,816 A  | 3/1999  | Wright             | 6,619,400 B2 | 9/2003  | Brunet               |
| 5,896,819 A  | 4/1999  | Turila et al.      | 6,634,428 B2 | 10/2003 | Krauss et al.        |
| 5,902,424 A  | 5/1999  | Fujita et al.      | 6,662,886 B2 | 12/2003 | Russell              |
| 5,934,372 A  | 8/1999  | Muth               | 6,675,889 B1 | 1/2004  | Mullins et al.       |
| 5,960,881 A  | 10/1999 | Allamon et al.     | 6,699,305 B2 | 3/2004  | Myrick               |
| 5,990,051 A  | 11/1999 | Ischy et al.       | 6,713,177 B2 | 3/2004  | George et al.        |
| 5,992,452 A  | 11/1999 | Nelson, II         | 6,715,541 B2 | 4/2004  | Pedersen et al.      |
| 5,992,520 A  | 11/1999 | Schultz et al.     | 6,719,051 B2 | 4/2004  | Hailey, Jr. et al.   |
| 6,007,314 A  | 12/1999 | Nelson, II         | 6,755,249 B2 | 6/2004  | Robison et al.       |
| 6,024,915 A  | 2/2000  | Kume et al.        | 6,776,228 B2 | 8/2004  | Pedersen et al.      |
| 6,032,735 A  | 3/2000  | Echols             | 6,779,599 B2 | 8/2004  | Mullins et al.       |
| 6,036,777 A  | 3/2000  | Sachs              | 6,799,638 B2 | 10/2004 | Butterfield, Jr.     |
| 6,047,773 A  | 4/2000  | Zeltmann et al.    | 6,810,960 B2 | 11/2004 | Pia                  |
| 6,050,340 A  | 4/2000  | Scott              | 6,817,414 B2 | 11/2004 | Lee                  |
| 6,069,313 A  | 5/2000  | Kay                | 6,831,044 B2 | 12/2004 | Constien             |
| 6,076,600 A  | 6/2000  | Vick, Jr. et al.   | 6,883,611 B2 | 4/2005  | Smith et al.         |
| 6,079,496 A  | 6/2000  | Hirth              | 6,887,297 B2 | 5/2005  | Winter et al.        |
| 6,085,837 A  | 7/2000  | Massinon et al.    | 6,896,049 B2 | 5/2005  | Moyes                |
| 6,095,247 A  | 8/2000  | Streich et al.     | 6,896,061 B2 | 5/2005  | Hriscu et al.        |
| 6,119,783 A  | 9/2000  | Parker et al.      | 6,899,176 B2 | 5/2005  | Hailey, Jr. et al.   |
| 6,142,237 A  | 11/2000 | Christmas et al.   | 6,899,777 B2 | 5/2005  | Vaidyanathan et al.  |
| 6,161,622 A  | 12/2000 | Robb et al.        | 6,908,516 B2 | 6/2005  | Hehmann et al.       |
| 6,167,970 B1 | 1/2001  | Stout et al.       | 6,913,827 B2 | 7/2005  | George et al.        |
| 6,170,583 B1 | 1/2001  | Boyce              | 6,926,086 B2 | 8/2005  | Patterson et al.     |
| 6,173,779 B1 | 1/2001  | Smith              | 6,932,159 B2 | 8/2005  | Hovem                |
| 6,189,616 B1 | 2/2001  | Gano et al.        | 6,945,331 B2 | 9/2005  | Patel                |
| 6,213,202 B1 | 4/2001  | Read, Jr.          | 6,951,331 B2 | 10/2005 | Haughom et al.       |
| 6,220,350 B1 | 4/2001  | Brothers et al.    | 6,959,759 B2 | 11/2005 | Doane et al.         |
| 6,220,357 B1 | 4/2001  | Carmichael         | 6,973,970 B2 | 12/2005 | Johnston et al.      |
| 6,228,904 B1 | 5/2001  | Yadav et al.       | 6,973,973 B2 | 12/2005 | Howard et al.        |
| 6,237,688 B1 | 5/2001  | Burleson et al.    | 6,983,796 B2 | 1/2006  | Bayne et al.         |
| 6,238,280 B1 | 5/2001  | Ritt et al.        | 6,986,390 B2 | 1/2006  | Doane et al.         |
| 6,241,021 B1 | 6/2001  | Bowling            | 7,013,989 B2 | 3/2006  | Hammond et al.       |
| 6,248,399 B1 | 6/2001  | Hehmann            | 7,017,664 B2 | 3/2006  | Walker et al.        |
| 6,250,392 B1 | 6/2001  | Muth               | 7,017,677 B2 | 3/2006  | Keshavan et al.      |
| 6,273,187 B1 | 8/2001  | Voisin, Jr. et al. | 7,021,389 B2 | 4/2006  | Bishop et al.        |
| 6,276,452 B1 | 8/2001  | Davis et al.       | 7,025,146 B2 | 4/2006  | King et al.          |
| 6,276,457 B1 | 8/2001  | Moffatt et al.     | 7,028,778 B2 | 4/2006  | Krywitsky            |
| 6,279,656 B1 | 8/2001  | Sinclair et al.    | 7,044,230 B2 | 5/2006  | Starr et al.         |
| 6,287,445 B1 | 9/2001  | Lashmore et al.    | 7,049,272 B2 | 5/2006  | Sinclair et al.      |
| 6,302,205 B1 | 10/2001 | Ryll               | 7,051,805 B2 | 5/2006  | Doane et al.         |
| 6,315,041 B1 | 11/2001 | Carlisle et al.    | 7,059,410 B2 | 6/2006  | Bousche et al.       |
| 6,315,050 B2 | 11/2001 | Vaynshteyn et al.  | 7,090,027 B1 | 8/2006  | Williams             |
| 6,325,148 B1 | 12/2001 | Trahan et al.      | 7,093,664 B2 | 8/2006  | Todd et al.          |
| 6,328,110 B1 | 12/2001 | Joubert            | 7,096,945 B2 | 8/2006  | Richards et al.      |
| 6,341,653 B1 | 1/2002  | Firmaniuk et al.   | 7,096,946 B2 | 8/2006  | Jasser et al.        |
| 6,349,766 B1 | 2/2002  | Bussear et al.     | 7,097,906 B2 | 8/2006  | Gardner              |
| 6,354,379 B2 | 3/2002  | Miszewski et al.   | 7,108,080 B2 | 9/2006  | Tessari et al.       |
| 6,357,332 B1 | 3/2002  | Vecchio            | 7,111,682 B2 | 9/2006  | Blaisdell            |
| 6,371,206 B1 | 4/2002  | Mills              | 7,141,207 B2 | 11/2006 | Jandeska, Jr. et al. |
| 6,372,346 B1 | 4/2002  | Toth               | 7,150,326 B2 | 12/2006 | Bishop et al.        |
| 6,382,244 B2 | 5/2002  | Vann               | 7,163,066 B2 | 1/2007  | Lehr                 |
| 6,390,195 B1 | 5/2002  | Nguyen et al.      | 7,174,963 B2 | 2/2007  | Bertelsen            |
| 6,390,200 B1 | 5/2002  | Allamon et al.     | 7,182,135 B2 | 2/2007  | Szarka               |
| 6,394,185 B1 | 5/2002  | Constien           | 7,188,559 B1 | 3/2007  | Vecchio              |
| 6,397,950 B1 | 6/2002  | Streich et al.     | 7,210,527 B2 | 5/2007  | Walker et al.        |
| 6,408,946 B1 | 6/2002  | Marshall et al.    | 7,210,533 B2 | 5/2007  | Starr et al.         |
| 6,419,023 B1 | 7/2002  | George et al.      | 7,217,311 B2 | 5/2007  | Hong et al.          |
| 6,439,313 B1 | 8/2002  | Thomeer et al.     | 7,234,530 B2 | 6/2007  | Gass                 |
| 6,457,525 B1 | 10/2002 | Scott              | 7,252,162 B2 | 8/2007  | Akinlade et al.      |
| 6,467,546 B2 | 10/2002 | Allamon et al.     | 7,255,178 B2 | 8/2007  | Johnson              |
| 6,470,965 B1 | 10/2002 | Winzer             | 7,264,060 B2 | 9/2007  | Slup et al.          |
| 6,491,097 B1 | 12/2002 | ONeal et al.       | 7,267,172 B2 | 9/2007  | Hofman               |
|              |         |                    | 7,267,178 B2 | 9/2007  | Krywitsky            |
|              |         |                    | 7,270,186 B2 | 9/2007  | Johnson              |
|              |         |                    | 7,287,592 B2 | 10/2007 | Surjaatmadja et al.  |

(56)

## References Cited

## U.S. PATENT DOCUMENTS

|                |         |                           |                 |         |                      |
|----------------|---------|---------------------------|-----------------|---------|----------------------|
| 7,311,152 B2   | 12/2007 | Howard et al.             | 7,828,055 B2    | 11/2010 | Willauer et al.      |
| 7,316,274 B2   | 1/2008  | Xu et al.                 | 7,833,944 B2    | 11/2010 | Munoz et al.         |
| 7,320,365 B2   | 1/2008  | Pia                       | 7,849,927 B2    | 12/2010 | Herrera              |
| 7,322,412 B2   | 1/2008  | Badalamenti et al.        | 7,855,168 B2    | 12/2010 | Fuller et al.        |
| 7,322,417 B2   | 1/2008  | Rytlewski et al.          | 7,861,779 B2    | 1/2011  | Vestavik             |
| 7,325,617 B2   | 2/2008  | Murray                    | 7,861,781 B2    | 1/2011  | D'Arcy               |
| 7,328,750 B2   | 2/2008  | Swor et al.               | 7,874,365 B2    | 1/2011  | East, Jr. et al.     |
| 7,331,388 B2   | 2/2008  | Vilela et al.             | 7,878,253 B2    | 2/2011  | Stowe et al.         |
| 7,337,854 B2   | 3/2008  | Horn et al.               | 7,896,091 B2    | 3/2011  | Williamson et al.    |
| 7,346,456 B2   | 3/2008  | Le Bemadjiel              | 7,897,063 B1    | 3/2011  | Perry et al.         |
| 7,360,593 B2   | 4/2008  | Constien                  | 7,900,696 B1    | 3/2011  | Nish et al.          |
| 7,360,597 B2   | 4/2008  | Blaisdell                 | 7,900,703 B2    | 3/2011  | Clark et al.         |
| 7,384,443 B2   | 6/2008  | Mirchandani               | 7,909,096 B2    | 3/2011  | Clark et al.         |
| 7,387,158 B2   | 6/2008  | Murray et al.             | 7,909,104 B2    | 3/2011  | Bjorgum              |
| 7,387,165 B2   | 6/2008  | Lopez de Cardenas et al.  | 7,909,110 B2    | 3/2011  | Sharma et al.        |
| 7,392,841 B2   | 7/2008  | Murray et al.             | 7,909,115 B2    | 3/2011  | Grove et al.         |
| 7,401,648 B2   | 7/2008  | Richard                   | 7,958,940 B2    | 6/2011  | Crow et al.          |
| 7,416,029 B2   | 8/2008  | Telfer et al.             | 7,963,331 B2    | 6/2011  | Surjaatmadja et al.  |
| 7,422,058 B2   | 9/2008  | O'Malley                  | 7,963,340 B2    | 6/2011  | Gramstad et al.      |
| 7,426,964 B2   | 9/2008  | Lynde et al.              | 7,963,342 B2    | 6/2011  | George               |
| 7,441,596 B2   | 10/2008 | Wood et al.               | 7,980,300 B2    | 7/2011  | Roberts et al.       |
| 2,080,277 A1   | 11/2008 | Koda et al.               | 7,987,906 B1    | 8/2011  | Troy                 |
| 7,445,049 B2   | 11/2008 | Howard et al.             | 7,992,763 B2    | 8/2011  | Vecchio et al.       |
| 7,451,815 B2   | 11/2008 | Hailey, Jr.               | 8,020,619 B1    | 9/2011  | Robertson et al.     |
| 7,451,817 B2   | 11/2008 | Reddy et al.              | 8,020,620 B2    | 9/2011  | Daniels et al.       |
| 7,461,699 B2   | 12/2008 | Richard et al.            | 8,025,104 B2    | 9/2011  | Cooke, Jr.           |
| 7,464,764 B2   | 12/2008 | Xu                        | 8,028,767 B2    | 10/2011 | Radford et al.       |
| 7,472,750 B2   | 1/2009  | Walker et al.             | 8,033,331 B2    | 10/2011 | Themig               |
| 7,478,676 B2   | 1/2009  | East, Jr. et al.          | 8,039,422 B1    | 10/2011 | Al-Zahrani           |
| 7,503,390 B2   | 3/2009  | Gomez                     | 8,056,628 B2    | 11/2011 | Whitsitt et al.      |
| 7,503,399 B2   | 3/2009  | Badalamenti et al.        | 8,056,638 B2    | 11/2011 | Clayton et al.       |
| 7,510,018 B2   | 3/2009  | Williamson et al.         | 8,109,340 B2    | 2/2012  | Doane et al.         |
| 7,513,311 B2   | 4/2009  | Gramstad et al.           | 8,127,856 B1    | 3/2012  | Nish et al.          |
| 7,527,103 B2   | 5/2009  | Huang et al.              | 8,153,052 B2    | 4/2012  | Jackson et al.       |
| 7,537,825 B1   | 5/2009  | Wardle et al.             | 8,163,060 B2    | 4/2012  | Imanishi et al.      |
| 7,552,777 B2   | 6/2009  | Murray et al.             | 8,211,247 B2    | 7/2012  | Marya et al.         |
| 7,552,779 B2   | 6/2009  | Murray                    | 8,211,248 B2    | 7/2012  | Marya                |
| 7,575,062 B2   | 8/2009  | East, Jr.                 | 8,226,740 B2    | 7/2012  | Chaumonnot et al.    |
| 7,591,318 B2   | 9/2009  | Tilghman                  | 8,230,731 B2    | 7/2012  | Dyer et al.          |
| 7,600,572 B2   | 10/2009 | Slup et al.               | 8,231,947 B2    | 7/2012  | Vaidya et al.        |
| 7,604,055 B2   | 10/2009 | Richard et al.            | 8,276,670 B2    | 10/2012 | Patel                |
| 7,617,871 B2   | 11/2009 | Surjaatmadja et al.       | 8,277,974 B2    | 10/2012 | Kumar et al.         |
| 7,635,023 B2   | 12/2009 | Goldberg et al.           | 8,297,364 B2    | 10/2012 | Agrawal et al.       |
| 7,640,988 B2   | 1/2010  | Phi et al.                | 8,327,931 B2    | 12/2012 | Agrawal et al.       |
| 7,661,480 B2   | 2/2010  | Al-Anazi                  | 8,403,037 B2    | 3/2013  | Agrawal et al.       |
| 7,661,481 B2   | 2/2010  | Todd et al.               | 8,425,651 B2    | 4/2013  | Xu et al.            |
| 7,665,537 B2   | 2/2010  | Patel et al.              | 2001/0045285 A1 | 11/2001 | Russell              |
| 7,686,082 B2   | 3/2010  | Marsh                     | 2001/0045288 A1 | 11/2001 | Allamont et al.      |
| 7,690,436 B2   | 4/2010  | Turley et al.             | 2002/0000319 A1 | 1/2002  | Brunet               |
| 7,699,101 B2 * | 4/2010  | Fripp et al. .... 166/229 | 2002/0007948 A1 | 1/2002  | Bayne et al.         |
| 7,703,510 B2   | 4/2010  | Xu                        | 2002/0014268 A1 | 2/2002  | Vann                 |
| 7,703,511 B2   | 4/2010  | Buyers et al.             | 2002/0066572 A1 | 6/2002  | Muth                 |
| 7,708,078 B2   | 5/2010  | Stoesz                    | 2002/0104616 A1 | 8/2002  | De et al.            |
| 7,709,421 B2   | 5/2010  | Jones et al.              | 2002/0136904 A1 | 9/2002  | Glass et al.         |
| 7,712,541 B2   | 5/2010  | Loretz et al.             | 2002/0162661 A1 | 11/2002 | Krauss et al.        |
| 7,723,272 B2   | 5/2010  | Crews et al.              | 2003/0037925 A1 | 2/2003  | Walker et al.        |
| 7,726,406 B2   | 6/2010  | Xu                        | 2003/0060374 A1 | 3/2003  | Cooke, Jr.           |
| 7,735,578 B2   | 6/2010  | Loehr et al.              | 2003/0075326 A1 | 4/2003  | Ebinger              |
| 7,752,971 B2   | 7/2010  | Loehr                     | 2003/0104147 A1 | 6/2003  | Bretschneider et al. |
| 7,757,773 B2   | 7/2010  | Rytlewski                 | 2003/0111728 A1 | 6/2003  | Thai et al.          |
| 7,762,342 B2   | 7/2010  | Richard et al.            | 2003/0127013 A1 | 7/2003  | Zavitsanos et al.    |
| 7,770,652 B2   | 8/2010  | Barnett                   | 2003/0141060 A1 | 7/2003  | Hailey et al.        |
| 7,775,284 B2   | 8/2010  | Richards et al.           | 2003/0141061 A1 | 7/2003  | Hailey et al.        |
| 7,775,285 B2   | 8/2010  | Surjaatmadja et al.       | 2003/0141079 A1 | 7/2003  | Doane et al.         |
| 7,775,286 B2   | 8/2010  | Duphorne                  | 2003/0150614 A1 | 8/2003  | Brown et al.         |
| 7,784,543 B2   | 8/2010  | Johnson                   | 2003/0155114 A1 | 8/2003  | Pedersen et al.      |
| 7,793,714 B2   | 9/2010  | Johnson                   | 2003/0155115 A1 | 8/2003  | Pedersen et al.      |
| 7,798,225 B2   | 9/2010  | Giroux et al.             | 2003/0159828 A1 | 8/2003  | Howard et al.        |
| 7,798,226 B2   | 9/2010  | Themig                    | 2003/0164237 A1 | 9/2003  | Butterfield          |
| 7,798,236 B2   | 9/2010  | McKeachnie et al.         | 2003/0183391 A1 | 10/2003 | Hriscu et al.        |
| 7,806,189 B2   | 10/2010 | Frazier                   | 2004/0005483 A1 | 1/2004  | Lin                  |
| 7,806,192 B2   | 10/2010 | Foster et al.             | 2004/0020832 A1 | 2/2004  | Richards et al.      |
| 7,810,553 B2   | 10/2010 | Cruickshank et al.        | 2004/0031605 A1 | 2/2004  | Mickey               |
| 7,810,567 B2   | 10/2010 | Daniels et al.            | 2004/0045723 A1 | 3/2004  | Slup et al.          |
| 7,819,198 B2   | 10/2010 | Birckhead et al.          |                 |         |                      |

| (56)                  | References Cited |                           |                   |         |                           |                 |  |
|-----------------------|------------------|---------------------------|-------------------|---------|---------------------------|-----------------|--|
| U.S. PATENT DOCUMENTS |                  |                           |                   |         |                           |                 |  |
| 2004/0055758 A1       | 3/2004           | Brezinski et al.          | 2007/0277979 A1   | 12/2007 | Todd et al.               |                 |  |
| 2004/0089449 A1       | 5/2004           | Walton et al.             | 2007/0284109 A1   | 12/2007 | East et al.               |                 |  |
| 2004/0154806 A1       | 8/2004           | Bode et al.               | 2007/0284112 A1   | 12/2007 | Magne et al.              |                 |  |
| 2004/0159428 A1       | 8/2004           | Hammond et al.            | 2007/0299510 A1   | 12/2007 | Venkatraman et al.        |                 |  |
| 2004/0182583 A1       | 9/2004           | Doane et al.              | 2008/0011473 A1   | 1/2008  | Wood et al.               |                 |  |
| 2004/0256109 A1       | 12/2004          | Johnson                   | 2008/0020923 A1   | 1/2008  | Debe et al.               |                 |  |
| 2004/0256157 A1       | 12/2004          | Tessari et al.            | 2008/0047707 A1   | 2/2008  | Boney et al.              |                 |  |
| 2004/0261993 A1       | 12/2004          | Nguyen                    | 2008/0060810 A9   | 3/2008  | Nguyen et al.             |                 |  |
| 2005/0034876 A1       | 2/2005           | Doane et al.              | 2008/0066923 A1   | 3/2008  | Xu                        |                 |  |
| 2005/0051329 A1       | 3/2005           | Blaisdell                 | 2008/0066924 A1   | 3/2008  | Xu                        |                 |  |
| 2005/0064247 A1       | 3/2005           | Sane et al.               | 2008/0072705 A1   | 3/2008  | Chaumonnot et al.         |                 |  |
| 2005/0069449 A1       | 3/2005           | Jackson et al.            | 2008/0078553 A1   | 4/2008  | George                    |                 |  |
| 2005/0102255 A1       | 5/2005           | Bultman                   | 2008/0099209 A1   | 5/2008  | Loretz et al.             |                 |  |
| 2005/0106316 A1       | 5/2005           | Rigney et al.             | 2008/0115932 A1   | 5/2008  | Cooke                     |                 |  |
| 2005/0126334 A1       | 6/2005           | Mirchandani               | 2008/0121390 A1   | 5/2008  | O'Malley et al.           |                 |  |
| 2005/0161224 A1       | 7/2005           | Starr et al.              | 2008/0135249 A1   | 6/2008  | Fripp et al.              |                 |  |
| 2005/0165149 A1       | 7/2005           | Chanak et al.             | 2008/0149325 A1   | 6/2008  | Crawford                  |                 |  |
| 2005/0194143 A1       | 9/2005           | Xu et al.                 | 2008/0149345 A1   | 6/2008  | Marya et al.              |                 |  |
| 2005/0199401 A1       | 9/2005           | Patel et al.              | 2008/0169105 A1   | 7/2008  | Williamson et al.         |                 |  |
| 2005/0205264 A1       | 9/2005           | Starr et al.              | 2008/0179060 A1   | 7/2008  | Surjaatmadja et al.       |                 |  |
| 2005/0205266 A1       | 9/2005           | Todd et al.               | 2008/0179104 A1   | 7/2008  | Zhang et al.              |                 |  |
| 2005/0241824 A1       | 11/2005          | Burris, II et al.         | 2008/0202764 A1   | 8/2008  | Clayton et al.            |                 |  |
| 2005/0241825 A1       | 11/2005          | Burris, II et al.         | 2008/0202814 A1   | 8/2008  | Lyons et al.              |                 |  |
| 2005/0257936 A1       | 11/2005          | Lehr                      | 2008/0210473 A1   | 9/2008  | Zhang et al.              |                 |  |
| 2005/0279501 A1       | 12/2005          | Surjaatmadja et al.       | 2008/0216383 A1   | 9/2008  | Pierick et al.            |                 |  |
| 2006/0012087 A1       | 1/2006           | Matsuda et al.            | 2008/0223586 A1   | 9/2008  | Barnett                   |                 |  |
| 2006/0045787 A1       | 3/2006           | Jandeska, Jr. et al.      | 2008/0223587 A1   | 9/2008  | Cherewyk                  |                 |  |
| 2006/0057479 A1       | 3/2006           | Niimi et al.              | 2008/0236829 A1   | 10/2008 | Lynde                     |                 |  |
| 2006/0081378 A1       | 4/2006           | Howard et al.             | 2008/0248205 A1   | 10/2008 | Blanchet et al.           |                 |  |
| 2006/0102871 A1       | 5/2006           | Wang et al.               | 2008/0277109 A1   | 11/2008 | Vaidya                    |                 |  |
| 2006/0108114 A1       | 5/2006           | Johnson et al.            | 2008/0277980 A1   | 11/2008 | Koda et al.               |                 |  |
| 2006/0108126 A1       | 5/2006           | Horn et al.               | 2008/0282924 A1   | 11/2008 | Saenger et al.            |                 |  |
| 2006/0116696 A1       | 6/2006           | Odermatt et al.           | 2008/0296024 A1   | 12/2008 | Huang et al.              |                 |  |
| 2006/0124310 A1       | 6/2006           | Lopez de Cardenas         | 2008/0314581 A1   | 12/2008 | Brown                     |                 |  |
| 2006/0124312 A1       | 6/2006           | Rytlewski et al.          | 2008/0314588 A1   | 12/2008 | Langlais et al.           |                 |  |
| 2006/0131011 A1       | 6/2006           | Lynde et al.              | 2009/0044946 A1   | 2/2009  | Schasteen et al.          |                 |  |
| 2006/0131081 A1       | 6/2006           | Mirchandani et al.        | 2009/0044949 A1   | 2/2009  | King et al.               |                 |  |
| 2006/0144515 A1       | 7/2006           | Tada et al.               | 2009/0050334 A1 * | 2/2009  | Marya et al. .... 166/376 |                 |  |
| 2006/0150770 A1       | 7/2006           | Freim, III et al.         | 2009/0056934 A1   | 3/2009  | Xu                        |                 |  |
| 2006/0151178 A1       | 7/2006           | Howard et al.             | 2009/0065216 A1   | 3/2009  | Frazier                   |                 |  |
| 2006/0162927 A1       | 7/2006           | Walker et al.             | 2009/0084553 A1   | 4/2009  | Rytlewski et al.          |                 |  |
| 2006/0169453 A1       | 8/2006           | Savery et al.             | 2009/0084556 A1   | 4/2009  | Richards et al.           |                 |  |
| 2006/0207763 A1       | 9/2006           | Hofman et al.             | 2009/0090440 A1   | 4/2009  | Kellett et al.            |                 |  |
| 2006/0213670 A1       | 9/2006           | Bishop et al.             | 2009/0107684 A1   | 4/2009  | Cooke                     |                 |  |
| 2006/0231253 A1       | 10/2006          | Vilela et al.             | 2009/0114381 A1   | 5/2009  | Stroobants                |                 |  |
| 2006/0283592 A1       | 12/2006          | Sierra et al.             | 2009/0114382 A1   | 5/2009  | Grove et al.              |                 |  |
| 2007/0017674 A1       | 1/2007           | Blaisdell                 | 2009/0145666 A1   | 6/2009  | Radford et al.            |                 |  |
| 2007/0017675 A1       | 1/2007           | Hammami et al.            | 2009/0151949 A1   | 6/2009  | Marya et al.              |                 |  |
| 2007/0029082 A1       | 2/2007           | Giroux et al.             | 2009/0155616 A1   | 6/2009  | Thamida et al.            |                 |  |
| 2007/0039741 A1       | 2/2007           | Hailey                    | 2009/0159289 A1   | 6/2009  | Avant et al.              |                 |  |
| 2007/0044966 A1       | 3/2007           | Davies et al.             | 2009/0178808 A1   | 7/2009  | Williamson et al.         |                 |  |
| 2007/0051521 A1       | 3/2007           | Fiike et al.              | 2009/0194273 A1   | 8/2009  | Surjaatmadja et al.       |                 |  |
| 2007/0053785 A1       | 3/2007           | Hetz et al.               | 2009/0205841 A1   | 8/2009  | Kluge et al.              |                 |  |
| 2007/0054101 A1       | 3/2007           | Sigalas et al.            | 2009/0226704 A1   | 9/2009  | Kauppinen et al.          |                 |  |
| 2007/0057415 A1       | 3/2007           | Katagiri et al.           | 2009/0242202 A1   | 10/2009 | Rispler et al.            |                 |  |
| 2007/0062644 A1       | 3/2007           | Nakamura et al.           | 2009/0242208 A1   | 10/2009 | Bolding                   |                 |  |
| 2007/0074601 A1       | 4/2007           | Hong et al.               | 2009/0242214 A1   | 10/2009 | Foster et al.             |                 |  |
| 2007/0074873 A1       | 4/2007           | McKeachnie et al.         | 2009/0255667 A1   | 10/2009 | Clem et al.               |                 |  |
| 2007/0072199 A1       | 5/2007           | Smith et al.              | 2009/0255684 A1   | 10/2009 | Bolding                   |                 |  |
| 2007/0107899 A1       | 5/2007           | Werner et al.             | 2009/0255686 A1   | 10/2009 | Richard et al.            |                 |  |
| 2007/0107908 A1       | 5/2007           | Vaidya et al.             | 2009/0260817 A1   | 10/2009 | Gambier et al.            |                 |  |
| 2007/0108060 A1       | 5/2007           | Park                      | 2009/0266548 A1   | 10/2009 | Olsen et al.              |                 |  |
| 2007/0119600 A1       | 5/2007           | Slup et al.               | 2009/0272544 A1   | 11/2009 | Giroux et al.             |                 |  |
| 2007/0131912 A1       | 6/2007           | Simone et al.             | 2009/0283270 A1   | 11/2009 | Langeslag                 |                 |  |
| 2007/0151009 A1       | 7/2007           | Conrad, III et al.        | 2009/0293672 A1   | 12/2009 | Mirchandani et al.        |                 |  |
| 2007/0151769 A1       | 7/2007           | Slutz et al.              | 2009/0301730 A1   | 12/2009 | Gweily                    |                 |  |
| 2007/0169935 A1       | 7/2007           | Akbar et al.              | 2009/0305131 A1   | 12/2009 | Kumar et al.              |                 |  |
| 2007/0181224 A1 *     | 8/2007           | Marya et al. .... 148/400 | 2010/0015469 A1   | 1/2010  | Howell et al.             |                 |  |
| 2007/0185655 A1       | 8/2007           | Le Bemadjiel              | 2010/0025255 A1   | 2/2010  | Macary                    |                 |  |
| 2007/0187095 A1       | 8/2007           | Walker et al.             | 2010/0032151 A1   | 2/2010  | Smith et al.              |                 |  |
| 2007/0221373 A1       | 9/2007           | Murray                    | 2010/0040180 A1   | 2/2010  | Dridahl et al.            |                 |  |
| 2007/0221384 A1       | 9/2007           | Murray                    | 2010/0044041 A1   | 2/2010  | Romanowski et al.         |                 |  |
| 2007/0261862 A1       | 11/2007          | Murray                    | 2010/0051278 A1   | 3/2010  | Su et al.                 |                 |  |
| 2007/0272411 A1       | 11/2007          | Lopez De Cardenas et al.  | 2010/0055491 A1   | 3/2010  | Duphorne                  |                 |  |
| 2007/0272413 A1       | 11/2007          | Rytlewski et al.          | 2010/0055492 A1   | 3/2010  | Kim et al.                |                 |  |
|                       |                  |                           |                   |         | 2/2010                    | Smith et al.    |  |
|                       |                  |                           |                   |         | 3/2010                    | Mytopher et al. |  |
|                       |                  |                           |                   |         | 3/2010                    | Vecchio et al.  |  |
|                       |                  |                           |                   |         | 3/2010                    | Barsoum et al.  |  |

| (56)                     | References Cited |                             | CN                                                                                                                                                                                                                                                                                                                                                                                               | 101457321 B   | 6/2010  |
|--------------------------|------------------|-----------------------------|--------------------------------------------------------------------------------------------------------------------------------------------------------------------------------------------------------------------------------------------------------------------------------------------------------------------------------------------------------------------------------------------------|---------------|---------|
| U.S. PATENT DOCUMENTS    |                  |                             |                                                                                                                                                                                                                                                                                                                                                                                                  |               |         |
| 2010/0089583 A1          | 4/2010           | Xu et al.                   | EP                                                                                                                                                                                                                                                                                                                                                                                               | 0033625 A1    | 8/1981  |
| 2010/0089587 A1          | 4/2010           | Stout                       | EP                                                                                                                                                                                                                                                                                                                                                                                               | 1857570 A2    | 11/2007 |
| 2010/0101803 A1          | 4/2010           | Clayton et al.              | GB                                                                                                                                                                                                                                                                                                                                                                                               | 912956        | 12/1962 |
| 2010/0122817 A1          | 5/2010           | Surjaatmadja et al.         | JP                                                                                                                                                                                                                                                                                                                                                                                               | 61067770      | 4/1986  |
| 2010/0139930 A1          | 6/2010           | Patel et al.                | JP                                                                                                                                                                                                                                                                                                                                                                                               | 7-54008       | 2/1995  |
| 2010/0200230 A1          | 8/2010           | East, Jr. et al.            | JP                                                                                                                                                                                                                                                                                                                                                                                               | 08232029      | 9/1996  |
| 2010/0236793 A1          | 9/2010           | Bjorgum                     | JP                                                                                                                                                                                                                                                                                                                                                                                               | 08-232029 A1  | 10/1996 |
| 2010/0236794 A1          | 9/2010           | Duan et al.                 | JP                                                                                                                                                                                                                                                                                                                                                                                               | 2010502840 A  | 1/2010  |
| 2010/0243254 A1          | 9/2010           | Murphy et al.               | KR                                                                                                                                                                                                                                                                                                                                                                                               | 95-0014350    | 11/1995 |
| 2010/0252273 A1          | 10/2010          | Duphorne                    | WO                                                                                                                                                                                                                                                                                                                                                                                               | 9947726 A1    | 9/1999  |
| 2010/0252280 A1          | 10/2010          | Swor et al.                 | WO                                                                                                                                                                                                                                                                                                                                                                                               | 2008034042 A3 | 3/2008  |
| 2010/0270031 A1          | 10/2010          | Patel                       | WO                                                                                                                                                                                                                                                                                                                                                                                               | 2008079777 A3 | 7/2008  |
| 2010/0276136 A1          | 11/2010          | Evans et al.                | WO                                                                                                                                                                                                                                                                                                                                                                                               | WO2008079485  | 7/2008  |
| 2010/0282338 A1          | 11/2010          | Gerrard et al.              | WO                                                                                                                                                                                                                                                                                                                                                                                               | 2009079745 A1 | 7/2009  |
| 2010/0282469 A1          | 11/2010          | Richard et al.              | WO                                                                                                                                                                                                                                                                                                                                                                                               | 2011071902 A3 | 6/2011  |
| 2010/0294510 A1          | 11/2010          | Holmes                      | WO                                                                                                                                                                                                                                                                                                                                                                                               | 2011071910 A2 | 6/2011  |
| 2010/0319870 A1          | 12/2010          | Bewlay et al.               | WO                                                                                                                                                                                                                                                                                                                                                                                               | 2012174101 A2 | 12/2012 |
| 2011/0005773 A1          | 1/2011           | Dusterhoff et al.           | WO                                                                                                                                                                                                                                                                                                                                                                                               | 2013053057 A1 | 4/2013  |
| 2011/0036592 A1          | 2/2011           | Fay                         | WO                                                                                                                                                                                                                                                                                                                                                                                               | 2013078031 A1 | 5/2013  |
| 2011/0048743 A1          | 3/2011           | Stafford et al.             | OTHER PUBLICATIONS                                                                                                                                                                                                                                                                                                                                                                               |               |         |
| 2011/0056692 A1          | 3/2011           | Lopez De Cardenas et al.    | Canadian Pat. App. No. 2783346 filed on Dec. 7, 2010, published on Jun. 16, 2011 for "Engineered Powder Compact Composite Material".                                                                                                                                                                                                                                                             |               |         |
| 2011/0056702 A1          | 3/2011           | Sharma et al.               | Flow Control Systems, [online]; [retrieved on May 20, 2010]; retrieved from the Internet <a href="http://www.bakerhughes.com/products-and-services/completions-and-productions/well-completions/packers-and-flow-control/flow-control-systems">http://www.bakerhughes.com/products-and-services/completions-and-productions/well-completions/packers-and-flow-control/flow-control-systems</a> . |               |         |
| 2011/0067872 A1          | 3/2011           | Agrawal                     | Optisleeve Sliding Sleeve, [online]; [retrieved on Jun. 25, 2010]; retrieved from the Internet <a href="http://weatherford.com/weatherford/groups/.../weatherfordecorp/WFT033159.pdf">weatherfordcorp/WFT033159.pdf</a> .                                                                                                                                                                        |               |         |
| 2011/0067889 A1          | 3/2011           | Marya et al.                | "Sliding Sleeve", Omega Completion Technology Ltd, Sep. 29, 2009, retrieved on: <a href="http://www.omega-completion.com">www.omega-completion.com</a> .                                                                                                                                                                                                                                         |               |         |
| 2011/0067890 A1          | 3/2011           | Themig                      | Welch, William R. et al., "Nonelastomeric Sliding Sleeve Maintains Long Term Integrity in HP/HT Application: Case Histories" [Abstract Only], SPE Eastern Regional Meeting, Oct. 23-25, 1996, Columbus, Ohio.                                                                                                                                                                                    |               |         |
| 2011/0094406 A1          | 4/2011           | Marya et al.                | Ambat, et al.; "Electroless Nickel-Plating on AZ91D Magnesium Alloy: Effect of Substrate Microstructure and Plating Parameters"; Surface and Coatings Technology; 179; pp. 124-134; (2004).                                                                                                                                                                                                      |               |         |
| 2011/0100643 A1          | 5/2011           | Themig et al.               | Chang, et al.; "Electrodeposition of Aluminum on Magnesium Alloy in Aluminum Chloride (A1C13)-1-ethy1-3-methylimidazolium chloride (EMIC) Ionic Liquid and Its Corrosion Behavior"; Electrochemistry Communications; 9; pp. 1602-1606; (2007).                                                                                                                                                   |               |         |
| 2011/0127044 A1          | 6/2011           | Radford et al.              | Chun-Lin, Li. "Design of Abrasive Water Jet Perforation and Hydraulic Fracturing Tool," Oil Field Equipment, Mar. 2011.                                                                                                                                                                                                                                                                          |               |         |
| 2011/0132621 A1 *        | 6/2011           | Agrawal et al. .... 166/376 | Forsyth, et al.; "An Ionic Liquid Surface Treatment for Corrosion Protection of Magnesium Alloy AZ31"; Electrochem. Solid-State Lett./ 9(11); Abstract only, 1 page.                                                                                                                                                                                                                             |               |         |
| 2011/0139465 A1          | 6/2011           | Tibbles et al.              | Forsyth, et al.; "Exploring Corrosion Protection of Mg Via Ionic Liquid Pretreatment"; Surface & Coatings Technology; 201; pp. 4496-4504; (2007).                                                                                                                                                                                                                                                |               |         |
| 2011/0147014 A1          | 6/2011           | Chen et al.                 | Hsiao et al.; "Effect of Heat Treatment on Anodization and Electrochemical Behavior of AZ91D Magnesium Alloy"; J. Mater. Res.; 20(10); pp. 2763-2771; (2005).                                                                                                                                                                                                                                    |               |         |
| 2011/0186306 A1          | 8/2011           | Marya et al.                | Hsiao, et al.; "Anodization of AZ91D Magnesium Alloy in Silicate-Containing Electrolytes"; Surface & Coatings Technology; 199; pp. 127-134; (2005).                                                                                                                                                                                                                                              |               |         |
| 2011/0214881 A1          | 9/2011           | Newton et al.               | Hsiao, et al.; "Baking Treatment Effect on Materials Characteristics and Electrochemical Behavior of anodic Film Formed on AZ91D Magnesium Alloy"; Corrosion Science; 49; pp. 781-793; (2007).                                                                                                                                                                                                   |               |         |
| 2011/0247833 A1          | 10/2011          | Todd et al.                 | Hsiao, et al.; "Characterization of Anodic Films Formed on AZ91D Magnesium Alloy"; Surface & Coatings Technology; 190; pp. 299-308; (2005).                                                                                                                                                                                                                                                      |               |         |
| 2011/0253387 A1          | 10/2011          | Ervin                       | Huo et al.; "Corrosion of AZ91D Magnesium Alloy with a Chemical Conversion Coating and Electroless Nickel Layer"; Corrosion Science; 46; pp. 1467-1477; (2004).                                                                                                                                                                                                                                  |               |         |
| 2011/0256356 A1          | 10/2011          | Tomantschger et al.         | Notification of Transmittal of the International Search Report and the Written Opinion of the International Searching Authority; PCT/US2010/059257; Korean Intellectual Property Office; Mailed Jul. 27, 2011.                                                                                                                                                                                   |               |         |
| 2011/0259610 A1          | 10/2011          | Shkurti et al.              | Page 6                                                                                                                                                                                                                                                                                                                                                                                           |               |         |
| 2011/0277987 A1          | 11/2011          | Frazier                     | Page 6                                                                                                                                                                                                                                                                                                                                                                                           |               |         |
| 2011/0277989 A1          | 11/2011          | Frazier                     | Page 6                                                                                                                                                                                                                                                                                                                                                                                           |               |         |
| 2011/0284232 A1          | 11/2011          | Huang                       | Page 6                                                                                                                                                                                                                                                                                                                                                                                           |               |         |
| 2011/0284240 A1          | 11/2011          | Chen et al.                 | Page 6                                                                                                                                                                                                                                                                                                                                                                                           |               |         |
| 2011/0284243 A1          | 11/2011          | Frazier                     | Page 6                                                                                                                                                                                                                                                                                                                                                                                           |               |         |
| 2011/0300403 A1          | 12/2011          | Vecchio et al.              | Page 6                                                                                                                                                                                                                                                                                                                                                                                           |               |         |
| 2012/0067426 A1          | 3/2012           | Soni et al.                 | Page 6                                                                                                                                                                                                                                                                                                                                                                                           |               |         |
| 2012/0103135 A1          | 5/2012           | Xu et al.                   | Page 6                                                                                                                                                                                                                                                                                                                                                                                           |               |         |
| 2012/0107590 A1          | 5/2012           | Xu et al.                   | Page 6                                                                                                                                                                                                                                                                                                                                                                                           |               |         |
| 2012/0118583 A1          | 5/2012           | Johnson et al.              | Page 6                                                                                                                                                                                                                                                                                                                                                                                           |               |         |
| 2012/0130470 A1          | 5/2012           | Agnew et al.                | Page 6                                                                                                                                                                                                                                                                                                                                                                                           |               |         |
| 2012/0145389 A1          | 6/2012           | Fitzpatrick, Jr.            | Page 6                                                                                                                                                                                                                                                                                                                                                                                           |               |         |
| 2012/0168152 A1          | 7/2012           | Casciaro                    | Page 6                                                                                                                                                                                                                                                                                                                                                                                           |               |         |
| 2012/0211239 A1          | 8/2012           | Kritzler et al.             | Page 6                                                                                                                                                                                                                                                                                                                                                                                           |               |         |
| 2012/0267101 A1          | 10/2012          | Cooke                       | Page 6                                                                                                                                                                                                                                                                                                                                                                                           |               |         |
| 2012/0292053 A1          | 11/2012          | Xu et al.                   | Page 6                                                                                                                                                                                                                                                                                                                                                                                           |               |         |
| 2012/0318513 A1 *        | 12/2012          | Mazyar et al. .... 166/304  | Page 6                                                                                                                                                                                                                                                                                                                                                                                           |               |         |
| 2013/0004847 A1          | 1/2013           | Kumar et al.                | Page 6                                                                                                                                                                                                                                                                                                                                                                                           |               |         |
| 2013/0025409 A1          | 1/2013           | Xu                          | Page 6                                                                                                                                                                                                                                                                                                                                                                                           |               |         |
| 2013/0032357 A1          | 2/2013           | Mazyar et al.               | Page 6                                                                                                                                                                                                                                                                                                                                                                                           |               |         |
| 2013/0048304 A1          | 2/2013           | Agrawal et al.              | Page 6                                                                                                                                                                                                                                                                                                                                                                                           |               |         |
| 2013/0052472 A1          | 2/2013           | Xu                          | Page 6                                                                                                                                                                                                                                                                                                                                                                                           |               |         |
| 2013/0081814 A1          | 4/2013           | Gaudette et al.             | Page 6                                                                                                                                                                                                                                                                                                                                                                                           |               |         |
| 2013/0105159 A1          | 5/2013           | Alvarez et al.              | Page 6                                                                                                                                                                                                                                                                                                                                                                                           |               |         |
| 2013/0126190 A1          | 5/2013           | Mazyar et al.               | Page 6                                                                                                                                                                                                                                                                                                                                                                                           |               |         |
| 2013/0133897 A1          | 5/2013           | Baihly et al.               | Page 6                                                                                                                                                                                                                                                                                                                                                                                           |               |         |
| 2013/0146144 A1          | 6/2013           | Joseph et al.               | Page 6                                                                                                                                                                                                                                                                                                                                                                                           |               |         |
| 2013/0146302 A1          | 6/2013           | Gaudette et al.             | Page 6                                                                                                                                                                                                                                                                                                                                                                                           |               |         |
| 2013/0186626 A1          | 7/2013           | Aitken et al.               | Page 6                                                                                                                                                                                                                                                                                                                                                                                           |               |         |
| 2013/0240203 A1          | 9/2013           | Frazier                     | Page 6                                                                                                                                                                                                                                                                                                                                                                                           |               |         |
| 2013/0327540 A1          | 12/2013          | Hamid et al.                | Page 6                                                                                                                                                                                                                                                                                                                                                                                           |               |         |
| 2014/0116711 A1          | 5/2014           | Tang et al.                 | Page 6                                                                                                                                                                                                                                                                                                                                                                                           |               |         |
| FOREIGN PATENT DOCUMENTS |                  |                             |                                                                                                                                                                                                                                                                                                                                                                                                  |               |         |
| CN                       | 101050417 A      | 10/2007                     | Page 6                                                                                                                                                                                                                                                                                                                                                                                           |               |         |
| CN                       | 101351523 A      | 1/2009                      | Page 6                                                                                                                                                                                                                                                                                                                                                                                           |               |         |

(56)

## References Cited

## OTHER PUBLICATIONS

- Liu, et al.; "Electroless Nickel Plating on AZ91 Mg Alloy Substrate"; *Surface & Coatings Technology*; 200; pp. 5087-5093; (2006).
- Lunder et al.; "The Role of Mg17Al12 Phase in the Corrosion of Mg Alloy AZ91"; *Corrosion*; 45(9); pp. 741-748; (1989).
- Pardo, et al.; "Corrosion Behaviour of Magnesium/Aluminium Alloys in 3.5 wt% NaCl"; *Corrosion Science*; 50; pp. 823-834; (2008).
- Shi et al.; "Influence of the Beta Phase on the Corrosion Performance of Anodised Coatings on Magnesium-Aluminium Alloys"; *Corrosion Science*; 47; pp. 2760-2777; (2005).
- Song, et al.; "Corrosion Mechanisms of Magnesium Alloys"; *Advanced Engineering Materials*; 1(1); pp. 11-33; (1999).
- Song, Guangling; "Recent Progress in Corrosion and Protection of Magnesium Alloys"; *Advanced Engineering Materials*; 7(7); pp. 563-586; (2005).
- Song, et al.; "Influence of Microstructure on the Corrosion of Diecast AZ91D"; *Corrosion Science*; 41; pp. 249-273; (1999).
- Song, et al.; "Corrosion Behaviour of AZ21, AZ501 and AZ91 in Sodium Chloride"; *Corrosion Science*; 40(10); pp. 1769-1791; (1998).
- Song et al.; "Understanding Magnesium Corrosion"; *Advanced Engineering Materials*; 5; No. 12; pp. 837-858; (2003).
- Zhang, et al.; "Study on the Environmentally Friendly Anodizing of AZ91D Magnesium Alloy"; *Surface and Coatings Technology*; 161; pp. 36-43; (2002).
- International Search Report and Written Opinion; Mail Date Jul. 28, 2011; International Application No. PCT/US2010/057763; International Filing date Nov. 23, 2010; Korean Intellectual Property Office; International Search Report 7 pages; Written Opinion 3 pages.
- H. Watarai, Trend of research and development for magnesium alloys-reducing the weight of structural materials in motor vehicles, (2006) *Science and technology trends*, Quaterly review No. 18, 84-97.
- M. Bououdina, Z. X. Guo, Comparative study of mechanical alloying of (Mg+Al) and (Mg+Al+Ni) mixtures for hydrogen storage, *J. Alloys, Compds*, 2002, 336, 222-231.
- M.Liu, P.J. Uggowitzer, A.V. Nagasekhar, P. Schmutz, M. Easton, G.L. Song, A. Atnens, Calculated phase diagrams and the corrosion of die-cast Mg-Al alloys, *Corrosion Science*, 2009, 51, 606-619.
- S.L. Lee, C.W. Hsu, F.K. Hsu, C.Y. Chou, C.K. Lin, C.W. Weng, Effects of Ni addition on hydrogen storage properties of Mg17Al12alloy, *Materials Chemistry and Physics*, 2011, 126, 319-324.
- T.J. Bastow, S. Celotto, Clustering and formation of nano-precipitates in dilute aluminum and magnesium alloys, *Materials science and Engineering*, 2003, C23, 757-762.
- Constantine, Jesse. "Selective Production of Horizontal Openhole Completions Using ECP and Sliding Sleeve Technology." SPE Rocky Mountain Regional Meeting, May 15-18, 1999, Gillette, Wyoming. [Abstract Only].
- Elsayed Ayman, Imai Hisashi, Umeda Junko and Kondoh Katsuyoshi, "Effect of Consolidation and Extrusion Temperatures on Tensile Properties of Hot Extruded ZK61 Magnesium Alloy Gas Atomized Powders via Spark Plasma Sintering" *Transacation of JWRI*, vol. 38, (2009) No. 2, pp. 31-35.
- Bing Q. Han, Enrique J. Lavernia and Farghali A. Mohamed, "Mechanical Properties of Nanostructured Materials", *Rev. Adv. Mater. Sci.* 9(2005) 1-16.
- International Search Report and Written Opinion for PCT Application No. PCT/US2012/044866, dated Jan. 2, 2013, pp. 1-9.
- International Search Report and Written Opinion, PCT/US2012/046231, Date of Mailing Jan. 29, 2013, Korean Intellectual Property Office, Written Opinion 6 pages, International Search Report 3 pages.
- Adam J. Maisano, "Cryomilling of Aluminum-Based and Magnesium-Based Metal Powders", Thesis, Virginia Tech, Jan. 13, 2006.
- Nie, Xiaowu. "Patents of Methods to Prepare Intermetallic Matrix Composites: A Review," *Recent Patents on Materials Science* 2008, vol. 1, pp. 232-240.
- International Search Report and Written Opinion, International Application No. PCT/US2012/049434, Date of Mailing Feb. 1, 2013, Korean Intellectual Property Office, Written Opinion 4 pages, International Search Report 3 pages.
- E.J. Lavenia, B.Q. Han, J.M. Schoenung: "Cryomilled nanostructured materials: Processing and properties", *Materials Science and Engineering A*, 493, (2008) 207-214.
- International Search Report and Written Opinion; International Application No. PCT/US2012/038622; International Filing Date: May 18, 2012; Date of Mailing Dec. 6, 2012; 12 pages.
- International Search Report and Written Opinion; International Application No. PCT/US2010/057763; International Filing date Nov. 23, 2010; Korean Intellectual Property Office; International Search Report 7 pages; Written Opinion 3 pages.
- International Search Report and Written Opinion; PCT/US2010/059257; Korean Intellectual Property Office; dated Jul. 27, 2011.
- Notification of Transmittal of The International Search Report and the Written Opinion of the International Searching Authority; PCT/US2010/059259; International Searching Authority KIPO; Mailed Jun. 13, 2011.
- International Search Report and Written Opinion, PCT/US2010/059263, dated Jul. 8, 2011.
- Notification of Transmittal of The International Search Report and the Written Opinion of the International Searching Authority; PCT/US2010/059265; International Searching Authority KIPO; Mailed Jun. 16, 2011.
- Notification of Transmittal of The International Search Report and the Written Opinion of the International Searching Authority; PCT/US2010/059268; International Searching Authority KIPO; Mailed Jun. 17, 2011.
- Notification of Transmittal of the International Search Report and the Written Opinion of the International Searching Authority, or the Declaration mailed on Feb. 23, 2012 (Dated Feb. 22, 2012) for PCT/US2011/043036.
- Notification of Transmittal of the International Search Report and the Written Opinion of the International Searching Authority; PCT/US2011/047000; Korean Intellectual Property Office; Mailed Dec. 26, 2011; 8 pages.
- International Search Report and Written Opinion of the International Searching Authority for International Application No. PCT/US2011/058099 (filed on Oct. 27, 2011), mailed on May 11, 2012.
- International Search Report and Written Opinion of the International Searching Authority, or the Declaration for PCT/US2011/058105 mailed from the Korean Intellectual Property Office on May 1, 2012.
- International Search Report and Written Opinion for International application No. PCT/US2012/034973 filed on Apr. 25, 2012, mailed on Nov. 29, 2012.
- Patent Cooperation Treaty International Search Report and Written Opinion for International Patent Application No. PCT/US2012/034978 filed on Apr. 25, 2012, mailed on Nov. 12, 2012.
- Shumbera et al. "Improved Water Injector Performance in a Gulf of Mexico Deepwater Development Using an Openhole Frac Pack Completion and Downhole Filter System: Case History." SPE Annual Technical Conference and Exhibition, Oct. 5-8, 2003, Denver, Colorado. [Abstract Only].
- Vickery, Harold and Christian Bayne, "New One-Trip Multi-Zone Frac Pack System with Positive Positioning." European Petroleum Conference, Oct. 29-31, 2002, Aberdeen, UK. [Abstract Only].
- H. Watanabe, T. Mukai, M. Mabuchi and K. Higashi, "Superplastic Deformation Mechanism in Powder Metallurgy Magnesium Alloys and Composites", *Acta mater.* 49 (2001) pp. 2027-2037.
- Xiaowu Nie, Patents of Methods to Prepare Intermetallic Matrix Composites: A Review, *Recent Patents on Materials Science* 2008, 1, 232-240, Department of Scientific Research, Hunan Railway College of Science and Technology, Zhuzhou, P.R. China.
- Baker Oil Tools. "Z-Seal Metal-to-Metal Expandable Sealing Device Uses Expanding Metal in Place of Elastomers," Nov. 6, 2006.
- "Reactivity series", Wikipedia, [http://en.wikipedia.org/w/index.php?title=Reactivity\\_series&printable=yes](http://en.wikipedia.org/w/index.php?title=Reactivity_series&printable=yes) downloaded on May 18, 2014. 8 pages.
- Adams, et al.; "Thermal stabilities of aromatic acids as geothermal tracers", *Geothermics*, vol. 21, No. 3, 1992, pp. 323-339.

(56)

**References Cited****OTHER PUBLICATIONS**

- Canadian Office Action for Canadian Application No. 2,783,241, dated Feb. 25, 2013, pp. 1-3.
- Canadian Office Action for Canadian Application No. 2,783,346, dated Feb. 21, 2013, pp. 1-4.
- Canadian Office Action for Canadian Application No. 2,783,547, dated Feb. 15, 2013, pp. 1-3.
- Canadian Office Action for Canadian Application No. 2,833,958, dated Sep. 23, 2014, pp. 1-2.
- Canadian Office Action for Canadian Application No. 2,833,981, dated Sep. 23, 2014, pp. 1-2.
- Carrejo, et al., "Improving Flow Assurance in Multi-Zone Fracturing Treatments in Hydrocarbon Reservoirs with High Strength Corrodible Tripping Balls"; Society of Petroleum Engineers; SPE Paper No. 151613; Apr. 16, 2012; 6 pages.
- Chinese Office Action for Chinese Application No. 201080055613.5, dated Nov. 4, 2014, pp. 1-20.
- Chinese Office Action for Chinese Application No. 201180012447.5, dated Jul. 3, 2014, 7 pages.
- Chinese Office Action for Chinese Application No. 201180052095.6, dated Jul. 21, 2014, pp. 1-32.
- Feng, et al., "Electroless Plating of Carbon Nanotubes with Silver" Journal of Materials Science, 39, (2004) pp. 3241-3243.
- Flahaut, et al., "Carbon Nanotube-Metal-Oxide Nanocomposites: Microstructure, Electrical Conductivity and Mechanical Properties" Acta amter 48 (2000), pp. 3803-3812.
- Garfield, New One-Trip Sand-Control Completion System that Eliminates Formation Damage Resulting From conventional Perforating and Gravel-Pack Operations.; SPE Annual Technical Conference and Exhibition, Oct., Sep. 12, 2005.
- Garfield, et al., "Maximizing Inflow Performance in Soft Sand Completions Using New One-trip Sand Control Liner Completion Technology", SPE European Formation Damage Conference, May 25-27, 2005.
- Goh, et al., "Development of novel carbon nanotube reinforced magnesium nanocomposites using the powder metallurgy technique", Nanotechnology 17 (2006) 7-12.
- International Search Report and Written Opinion; International Application No. PCT/US2012/053339; International Filing Date: Aug. 31, 2012; Date of Mailing: Feb. 15, 2013; 11 pages.
- International Search Report and Written Opinion; International Application No. PCT/US2012/053342; International Filing Date: Aug. 31, 2012; Date of Mailing: Feb. 19, 2013; 9 pages.
- International Search Report and Written Opinion; International Application No. PCT/US2012/053350; International Filing Date: Aug. 31, 2012; Date of Mailing: Feb. 25, 2013; 10 pages.
- International Search Report and Written Opinion; International Application No. PCT/US2014/049347; International Filing Date: Aug. 1, 2014; Date of Mailing: Nov. 24, 2014; 11 pages.
- International Search Report and Written Opinion; International Application No. PCT/US2014/054720; International Filing Date: Sep. 9, 2014; Date of Mailing: Dec. 17, 2014; 10 pages.
- Li, et al.; "Investigation of aluminium-based nanocomposites with ultra-high strength", Materials Science and Engineering A, 527, pp. 305-316, (2009).
- Mathis, "Sand Management: A Review of Approaches and Concerns", Society of Petroleum Engineers, SPE Paper No. 82240, SPE European Formation Damage Conference, The Hague, The Netherlands, May 13-14, 2003.
- Rose, et al.; "The application of the polycyclic aromatic sulfonates as tracers in geothermal reservoirs", Geothermics 30 (2001) pp. 617-640.
- Seyni, et al., "On the interest of using degradable fillers in co-ground composite materials", Powder Technology 190, (2009) pp. 176-184.
- Shaw, "Benefits and Application of a Surface-Controlled Sliding Sleeve for Fracturing Operations"; Society of Petroleum Engineers, SPE Paper No. 147546; Oct. 30, 2011; 8 pages.
- Shigematsu, et al., "Surface Treatment of AZ91D Magnesium Alloy by Aluminum diffusion Coating", Journal of Materials Science Letters 19, 2000, pp. 473-475.
- Shimizu, et al., "Multi-walled carbon nanotube-reinforced magnesium alloy composites", Scripta Materialia, vol. 58, Issue 4, pp. 267-270.
- Singh, et al., "Extended Homogeneity Range of Intermetallic Phases in Mechanically Alloyed Mg-Al Alloys", Elsevier Sciences Ltd., Intemetallics 11, 2003, pp. 373-376.
- Stanley, et al.; "An Introduction to Ground-Water Tracers", Department of Hydrology and Water Resources, University of Arizona, Mar. 1985, pp. 1-219.
- Sun, et al.; "Colloidal Processing of Carbon Nanotube/Alumina Composites" Chem. Mater. 2002, 14, pp. 5169-5172.
- Walters, et al.; "A Study of Jets from Unsintered-Powder Metal Lined Nonprecision Small-Caliber Shaped Charges", Army Research Laboratory, Aberdeen Proving Ground, MD 21005-5066; Feb. 2001.
- Xu, et al., "Nanostructured Material-Based Completion Tools Enhance Well Productivity"; International Petroleum Technology Conference; Conference Paper IPTC 16538; International Petroleum Technology Conference 2013; 4 pages.
- Zemel, "Tracers in the Oil Field", University of Texas at Austin, Center for Petroleum and Geosystems, Jan. 1995, Chapters 1, 2, 3, 7.
- Zhang, et al.; "High Strength Nanostructured Materials and Their Oil Field Applications"; Society of Petroleum Engineers, Conference Paper SPE 157092; SPE International Oilfield Nanotechnology Conference, 2012; 6 pages.
- International Search Report and Written Opinion; International Application No. PCT/US2012/071742; International Filing Date: Dec. 27, 2012; Date of Mailing: Apr. 22, 2013; 12 pages.
- International Search Report and Written Opinion; International Application No. PCT/US2014/058997, International Filing Date: Oct. 3, 2014; Date of Mailing: Jan. 12, 2015; 12 pages.
- International Search Report; International Application Application No. PCT/US2012/044229, International Filing Date: Jun. 26, 2012; Date of Mailing: Jan. 30, 2013; 3 pages.
- Murray, "Binary Alloy Phase Diagrams" Int. Met. Rev., 30(5) 1985 vol. 1, pp. 103-187.
- Vernon Constien et al., "Development of Reactive Coatings to Protect Sand-Control Screens", SPE 112494, Copyright 2008, Society of Petroleum Engineers, Presented at the 2008 SPE International Symposium and Exhibition on Formation Damage Control.
- Canadian Office Action for Canadian Application No. 2,834,794, dated Dec. 15, 2014, pp. 1-3.
- Danish Search Report and Opinion for Danish Application No. PA 2013 00060, dated Dec. 12, 2014, pp. 1-6.

\* cited by examiner

FIG. 1A



FIG. 1B



FIG. 1C



FIG. 2





**METHOD OF CONTROLLING CORROSION  
RATE IN DOWNHOLE ARTICLE, AND  
DOWNHOLE ARTICLE HAVING  
CONTROLLED CORROSION RATE**

**BACKGROUND**

Certain downhole operations involve placement of elements in a downhole environment, where the element performs its function, and is then removed. For example, elements such as ball/ball seat assemblies and fracture (frac) plugs are downhole elements used to seal off lower zones in a borehole in order to carry out a hydraulic fracturing process (also referred to in the art as "fracking") to break up different zones of reservoir rock. After the fracking operation, the ball/ball seat or plugs are then removed to allow fluid flow to or from the fractured rock.

Balls and/or ball seats, and frac plugs, can be formed of a corrodible material so that they need not be physically removed intact from the downhole environment. In this way, when the operation involving the ball/ball seat or frac plug is completed, the ball, ball seat, and/or frac plug is dissolved away. Otherwise, the downhole article may have to remain in the hole for a longer period than is necessary for the operation.

To facilitate removal, such elements can be formed of a material that reacts with the ambient downhole environment so that they need not be physically removed by, for example, a mechanical operation, but instead corrode or dissolve under downhole conditions. However, while corrosion rates of, for example, an alloy used to prepare such a corrodible article can be controlled by adjusting alloy composition, an alternative way of controlling the corrosion rate of a downhole article is desirable.

**SUMMARY**

The above and other deficiencies of the prior art are overcome by, in an embodiment, a method of removing a downhole assembly includes contacting, in the presence of an electrolyte, a first article including a first material and acting as an anode, and a second article including a second material having a lower reactivity than the first material and acting as a cathode, the downhole assembly including the first article in electrical contact with the second article, wherein at least a portion of the first article is corroded in the electrolyte.

In another embodiment, a method of producing an electrical potential in a downhole assembly includes contacting, with an electrolyte, a first article, the first article including a first material and acting as an anode, and a second article, the second article including a second material having a lower reactivity than the material of the first article and acting as a cathode, with a conductive element to form a circuit.

In another embodiment, a downhole assembly includes a first article including a first material and acting as an anode, and a second article including a second material having a lower reactivity than the first material and acting as a cathode, the first and second articles being electrically connected by a conductive element to form a circuit, wherein in the presence of an electrolyte, the downhole assembly produces an electrical potential, and at least a portion of the first article is corroded.

**BRIEF DESCRIPTION OF THE DRAWINGS**

Referring now to the drawings wherein like elements are numbered alike in the several Figures:

FIG. 1A shows a cross-sectional view of a downhole assembly 100a with a ball 120 made of a corrodible first metal, and a seat 110 having a seating portion 111 made of a second metal;

5 FIGS. 1B and 1C show a cross-sectional view of a downhole assembly (100b, 100c) with a ball 120 and a seat 111m shifting from a first position 110b to a second position 110c to place the seat 111m in contact with an insert 114 made of a second metal to initiate corrosion;

10 FIG. 2 shows a cross-sectional view of a downhole assembly 200 with a ball 220 with a core 221 made of a corrodible first metal, a coating 222, and a seat 210 having a seating portion 211 made of a second metal, in which a bridging connection B electrically connects the ball 220 and seat 210;

15 FIG. 3A shows a cross-sectional view of a downhole assembly 300 with a ball 320 with an axial core 321 of a first metal surrounded by an outer core 322, a seat 310 having a seating portion 311 made of a second metal; and

20 FIG. 3B shows a cross-sectional view of a downhole assembly 300a after removal of axial core 321 in FIG. 3A, with a ball 320a with a channel 321a surrounded by an outer core 322, and a seat 310 having a seating portion 311 made of a second metal.

**DETAILED DESCRIPTION OF THE INVENTION**

Disclosed herein is a method of controlling the corrosion of a downhole article. The downhole device includes an assembly of two subunits, a first subunit prepared from a first material, and a second subunit prepared from a second material, the first material having a higher galvanic activity (i.e., is more reactive) than the second material. The first and second materials can each be, for example, a different metal from the galvanic series. The first and second materials contact each 30 other in the presence of an electrolyte, such as for example brine. The first subunit is, for example, a ball, made of a corrodible, high reactivity metal such as magnesium, which is anodic, and the second subunit is, for example, a ball seat made of a non-corrodible, relatively low reactivity metal (as 35 compared to the high reactivity metal used to form the ball) such as nickel, iron, cobalt, etc, which is cathodic. Alternatively, in an embodiment, the first subunit is, for example, a ball seat, and the second, a ball. In an embodiment, by selecting the activities of the materials of the two subunits to have 40 a greater or lesser difference in corrosion potentials, the high reactivity material corrodes at a faster or slower rate, respectively.

To initiate galvanic corrosion, electrical coupling of the anodic high reactivity metal and cathodic low reactivity metal is required, and an electrolyte is also present and is at once in contact with both the anode and cathode. In an embodiment, electrically coupling these subunits initiates galvanic corrosion. Where the higher reactivity component (e.g., the ball) is 45 covered with a coating of an oxidation product of the high reactivity metal (such as Mg(OH)<sub>2</sub> where the high reactivity metal is magnesium or an alloy thereof), a direct current electrical potential can be applied to (or generated by) the anodic and cathodic subunits via the electrical connection, to initiate the corrosion of the subunit made of high reactivity metal (e.g., the ball). The direct current source can be, for 50 example, a battery placed downhole or at the surface, and electrically connected to the article.

Conversely, when these dissimilar metals are brought into 55 electrical contact in the presence of an electrolyte, an electrochemical potential is generated between the anodic high reactivity metal subunit (i.e., the ball in the above example) and the cathodic low reactivity metal subunit (e.g., a ball seat).

The greater the difference in corrosion potential between the dissimilar metals, the greater the electrical potential generated. In such an arrangement, the cathodic subunit is protected from corrosion by the anodic subunit, where the anodic subunit corrodes as a sacrificial anode. Corrosion of metal subunits in brines and other electrolytes can be reduced by coupling them to more active metals. For example, a steel article electrically coupled to a magnesium article in the presence of brine is less prone to corrosion than a steel article not in electrical contact with a magnesium article.

Electrically coupling the anodic ball and the cathodic ball seat with an electrolyte also produces an electrical potential useful to power a downhole device, such as, for example, a device for downhole signaling or sensing.

A method of removing a downhole assembly thus includes contacting, in the presence of an electrolyte, a first article comprising a first material and acting as an anode, and a second article comprising a second material having a lower reactivity than the material of the first article and acting as a cathode, the downhole assembly including the first article in electrical contact with the second article, wherein at least a portion of the first article is corroded in the electrolyte.

The first material includes any material suitable for use in a downhole environment, provided the first material is corrodible in the downhole environment relative to a second material having a different reactivity. In an embodiment, the first material comprises a magnesium alloy. Magnesium alloys include any such alloy which is corrodible in a corrosive environment including those typically encountered downhole, such as an aqueous environment which includes salt (i.e., brine), or an acidic or corrosive agent such as hydrogen sulfide, hydrochloric acid, or other such corrosive agents. Magnesium alloys suitable for use include alloys of magnesium with aluminum (Al), cadmium (Cd), calcium (Ca), cobalt (Co), copper (Cu), iron (Fe), manganese (Mn), nickel (Ni), silicon (Si), silver (Ag), strontium (Sr), thorium (Th), zinc (Zn), zirconium (Zr), or a combination comprising at least one of these elements. Particularly useful alloys include magnesium alloy particles including those prepared from magnesium alloyed with Ni, W, Co, Cu, Fe, or other metals. Alloying or trace elements can be included in varying amounts to adjust the corrosion rate of the magnesium. For example, four of these elements (cadmium, calcium, silver, and zinc) have to mild-to-moderate accelerating effects on corrosion rates, whereas four others (copper, cobalt, iron, and nickel) have a still greater accelerating effect on corrosion. Exemplary commercially available magnesium alloys which include different combinations of the above alloying elements to achieve different degrees of corrosion resistance include but are not limited to, for example, those alloyed with aluminum, strontium, and manganese such as AJ62, AJ50x, AJ51x, and AJ52x alloys, and those alloyed with aluminum, zinc, and manganese which include AZ91A-E alloys.

It will be appreciated that alloys having corrosion rates greater than those of the above exemplary alloys are contemplated as being useful herein. For example, nickel has been found to be useful in decreasing the corrosion resistance (i.e., increasing the corrosion rate) of magnesium alloys when included in amounts less than or equal to about 0.5 wt %, specifically less than or equal to about 0.4 wt %, and more specifically less than or equal to about 0.3 wt %, to provide a useful corrosion rate for the corrodible downhole article.

The above magnesium alloys are useful for forming the first article, and are formed into the desired shape and size by casting, forging and machining. Alternatively, powders of magnesium or the magnesium alloy are useful for forming the first article. The magnesium alloy powder generally has a

particle size of from about 50 to about 250 micrometers ( $\mu\text{m}$ ), and more specifically about 60 to about 140  $\mu\text{m}$ . The powder is further coated using a method such as chemical vapor deposition, anodization or the like, or admixed by physical method such as cryo-milling, ball milling, or the like, with a metal or metal oxide such as Al, Ni, W, Co, Cu, Fe, oxides of one of these metals, or the like. Such coated magnesium powders are referred to herein as controlled electrolytic materials (CEM). The CEM is then molded or compressed into the desired shape by, for example, cold compression using an isostatic press at about 40 to about 80 ksi (about 275 to about 550 MPa), followed by extrusion, forging, or sintering, or machining, to provide a core having the desired shape and dimensions.

It will be understood that the magnesium alloy or CEM, will thus have any corrosion rate necessary to achieve the desired performance of the article. In a specific embodiment, the magnesium alloy or CEM used to form the core has a corrosion rate of about 0.1 to about 150  $\text{mg}/\text{cm}^2/\text{hour}$ , specifically about 1 to about 15  $\text{mg}/\text{cm}^2/\text{hour}$  using aqueous 3 wt % KCl at 200° F. (93° C.).

The first article optionally has a non-metallic coating on a surface of the first article. The coating includes a soluble glass, a soluble polymer, or a metal oxide or hydroxide coating (including an anodized coating). In an embodiment, the non-metallic coating is an oxidation product of the metal of the first article, particularly where the first article comprises an active metal (relative to the second article). For example, where the first article comprises magnesium alloy, the non-metallic coating can be magnesium hydroxide formed by an anodic process. Alternatively, a hard metal oxide coating such as aluminum oxide can be applied to the surface of the first article by a deposition process.

The non-metallic coating is removed by ambient conditions downhole, or by application of an electric potential. For example, where the coating is a soluble material such as a soluble glass or polymer, the coating dissolves in the ambient downhole fluids, such as water, brine, distillates, or the like, to expose the underlying first material. Alternatively, where a metal oxide or hydroxide is used, an electrical contact can be established between the first and second articles, and an electrical potential applied to perform electrolysis on the coating and induce corrosion.

The second material is, in an embodiment, any metal having a lower reactivity than the first material, based on, for example, the saltwater galvanic series. The second material is also resistant to corrosion by a corrosive material. As used herein, "resistant" means the second material is not etched or corroded by any corrosive downhole conditions encountered (i.e., brine, hydrogen sulfide, etc., at pressures greater than atmospheric pressure, and at temperatures in excess of 50° C.).

By selecting the reactivity of the first and second materials to have a greater or lesser difference in their corrosion potentials, the high reactivity material (e.g., high reactivity metal) corrodes at a faster or slower rate, respectively. Generally, for metals in the galvanic series, the order of metals, from more noble (i.e., less active and more cathodic) to less noble (i.e., more active, and more anodic) includes for example steel, tungsten, chromium, nickel, cobalt, copper, iron, aluminum, zinc, and magnesium. The second material includes steel, tungsten, chromium, nickel, copper, iron, aluminum, zinc, alloys thereof, or a combination comprising at least one of the foregoing, where the first material is magnesium or an alloy thereof. In a specific embodiment, the first material is a magnesium alloy, and the second material is steel, nickel, cobalt, or copper.

In an embodiment, the second article is entirely fabricated of the second material, or the second article includes a layer of the second material. Here, a layer includes a single layer, or multiple layers of the same or different materials. Where layers are used, the underlying material is a metal, ceramic, or the like, and in an embodiment is, for example, fabricated from the first material such that it is separated from the first material of the first article by the layer(s) of second material.

The first article and second article are not limited to any particular shape or function. In an embodiment, the first and second articles are used together in a fitted assembly. For example, in one embodiment, the first article is CEM ball, and the second article is a ball seat. Alternatively, the first article is a CEM ball seat, and the second article is a ball. In another embodiment, the first article is a CEM fracture plug and the second is the housing for the fracture plug. In an embodiment, the first article is a CEM ball or frac plug, and the second article is the ball seat or housing (respectively), where this arrangement allows for greater adaptability of a system in which a variety of non-fixed articles (e.g., a ball) are all be used with one type of fixed article (such as a ball seat). Where desired, a portion of the fixed article (e.g., ball seat) is formed of a CEM coated with a more noble (second) metal such as zinc, aluminum, or nickel, so that the fixed article is removed by removing the second metal coating, and corroding the underlying CEM.

In an embodiment, the first article comprises a non-corrodible core comprising the second material and at least partially penetrating the first article, and a corrodible surrounding structure comprising the first material, wherein only the surrounding structure is corroded. The first article in this way is partially composed of the first material and second material. For example, the first article is a ball or elongated structure having one or more non-corrodible cores inserted part way into the article, or running axially or along a chord through the center of or off-center (respectively) of the ball or structure. Any dimension of the first article can be penetrated; in one embodiment, the longest dimension is traversed by the core. Thus, in an embodiment, the first article includes a low reactivity core (e.g., nickel) partially penetrating the first article, and a corrodible surrounding structure (e.g., a magnesium alloy or CEM).

In a non-limiting example, the first article is a corrodible ball formed of a magnesium alloy or CEM, having one or more nickel cores or screws inserted into it. This arrangement provides for close contact of the first and second materials, where the corrosion of the first article is accelerated by placing the article downhole and electrically connecting one or more of the nickel screws with the magnesium alloy ball. Conversely, the first article is a corrodible seat having one or more non-corrodible cores partially or fully penetrating (e.g., screwed) radially into the side. The presence of these cores provides additional contact between the first and second materials, and facilitates electrical contact with a second article (e.g., a ball where the first article is a seat, or vice versa).

In another embodiment, the first article comprises a corrodible core comprising the first material and at least partially penetrating the first article, and a non-corrodible surrounding structure comprising the second material, wherein only the core is corroded. The first article in this way includes a corrodible core penetrating through a long axis or diameter of the first article, and a non-corrodible surrounding structure. Application of a controlled corrosion to such first articles would then result in only the core being corroded, leaving a channel through the ball. In a non-limiting example, the first article is a non-corrodible ball made of a low reactivity mate-

rial (e.g., of aluminum or nickel), with one or more high reactivity (e.g., magnesium alloy) cores penetrating (e.g., screwed into or formed) therethrough.

Conversely, the first article is the seat having a corrodible core penetrating (e.g., screwed) radially through the side, where the corrosion and removal of the corrodible core opens to the underlying sidewall and any features (e.g., channels, etc) beneath. In this way, the ball (or seat) is used to allow a partial flow. In further embodiments, the core comprises more than one metal in successive layers, each having a different reactivity. This arrangement can be used to selectively increase the flow, such as by forming the first article of concentric layers of increasingly noble metals (on the galvanic scale, such as layers of different magnesium alloys, which are corrodible relative to the surrounding structure), which would allow a gradual increase in the size of the channel as additional layers are corroded.

The electrolyte includes an aqueous or non-aqueous electrolyte, depending on the application and controllability of ambient conditions. A non-aqueous electrolyte includes an ionic liquid, a molten salt, an ionic liquid dissolved in an oil, or a salt dissolved in a polar aprotic solvent such as ethylene carbonate, propylene carbonate, dimethylformamide, dimethylacetamide, gamma-butyrolactone, or other such solvents. However, where the article is a downhole element, controlling the ambient conditions to exclude moisture is not practical, and hence, under such conditions, the electrolyte is an aqueous electrolyte. Aqueous electrolytes include water or a salt dissolved in water, such as brine, an acid, or a combination comprising at least one of the foregoing.

In a method of controlling corrosion in a downhole environment, corroding the first article by the electrolyte is accomplished by electrically contacting the first and second articles in the presence of the electrolyte, optionally by inducing the corrosion by applying a potential to the first and second articles in the presence of the electrolyte. A direct current electrical potential can thus be applied to the anode and cathode (second and first articles, respectively, where the first and second articles are electrically insulated from one another and the cell is being run in reverse) via the electrical connection, to initiate the corrosion in the first article. The source of the direct current for this process can be, for example, a moving sleeve within the article, in which the sleeve is mechanically coupled to a power source (a battery, magneto, or a small generator which generates a current by induction).

In another embodiment, the downhole assembly, when electrically connected to provide a complete electrical circuit, produces electrical current by forming a galvanic cell in which the first and second articles (i.e., anode and cathode, comprising the first and second metals, respectively, where the cell is being run forward) are electrically connected by a bridging circuit in the presence of the electrolyte. The first and second articles are not in direct electrical contact with each other but are in electrical contact through (i.e., in common electrical contact with) an electrolyte, or where in physical contact are separated by, for example an insulating material such as a coating of  $Mg(OH)_2$  or a non-conductive O-ring to prevent a short circuit of the cell. Such an arrangement is sufficient to provide power to run a device such as for example, a transmitter or sensor, or other such device. Thus, a method of producing an electrical potential in a downhole assembly includes contacting, with an electrolyte, a first article, the first article comprising a first metal and acting as an anode; and a second article, the second article comprising a second metal having a lower reactivity than the metal of the first article and acting as a cathode. The anode and cathode are

in common electrical contact with each other via a conductive element (e.g., an electric load, such as a sensor or heater) to form a circuit.

A downhole assembly includes a first article comprising a first material, and a second article comprising a second material having a lower reactivity than the material of the first article and acting as a cathode, the first and second articles being electrically connected by a conductive element (e.g., electric load) to form a circuit, wherein in the presence of an electrolyte, the downhole assembly produces an electrical potential, and at least a portion of the first article is corroded.

Different exemplary embodiments of the downhole assembly are further described in the Figures.

FIG. 1A shows a cross-sectional view of a downhole assembly 100a. In the assembly 100a, a ball 120 made of a corrodible first metal is seated in a seat 110 having a seating portion 111 made of a second metal and contained in a housing 112. The ball 120 and seat 110 are in direct electrical contact with each other when an electrolyte is present, or where no insulating layer (such as Mg(OH)<sub>2</sub>) or other material separates ball 120 and seat 110.

In another embodiment, shown in FIGS. 1B and 1C, the ball 120 is seated in a movable seating portion 111m (initial assembly 100b in FIG. 1B). The seat 111m comprises the first metal, and is a movable unit held initially in a first position 110b in contact with the sidewall 113 not comprising a second metal. Upon seating ball 120 in the seat 111m, the seat 111m is shifted longitudinally through a surrounding housing 112 from the first position (110b in FIG. 1B), to a second position (110c in FIG. 1C) to provide the shifted assembly 100c in FIG. 1C, in which the seat 111m is in contact with an insert 114 formed of the second metal. In initial assembly 100b, insert 114 is electrically insulated from sidewall 113. In this way, the seat 111m is not corroded until it is moved into galvanic contact with the insert 114 of the second material. Also in an embodiment, the ball 120, seat 111m, and insert 114 are each formed of different materials of construction, where each is interchangeably made of the first metal, second metal, or a third metal having a reactivity intermediate to the first and second metals.

In another embodiment, FIG. 2 shows a cross-sectional view of a downhole assembly 200 with a ball 220 with a core 221 made of a corrodible first metal, a coating 222, and a seat 210 having a seating portion 211 made of a second metal and contained in a housing 212. In an embodiment, the coating is, for example, an oxidation product of the metal of the corrodible first metal (e.g., Mg(OH)<sub>2</sub> where the first metal is magnesium or a magnesium alloy). It will be appreciated that, in an embodiment, the presence of the coating electrically insulates the ball 220 from the seat 210, and hence, application of current by a power source electrically connected to a bridging connection (B) and which electrically connects the ball 220 and seat 210, initiates corrosion of ball 220, when an electrolyte is present.

In another example, FIG. 3A shows a cross-sectional view of a downhole assembly 300 with a ball 320 with an axial core 321 of a first metal surrounded by an outer core 322, a seat 310 having a seating portion 311 made of a second metal and housing 312. An optional bridging connection B (not shown) electrically connects the ball 320 and seat 310, and initiates corrosion of axial core 321 by application of current, where an insulative coating (not shown) is present, or generates a potential.

In another embodiment, the axial core 321 can be made of the first metal, while the outer core 322 can be made of the second metal, where the axial core 321 corrodes leaving the outer core 322. Similarly, in another embodiment, the axial

core 321 can be made of the second metal, while the outer core 322 can be made of the first metal, where the outer core 322 corrodes leaving the axial core 321. In these embodiments, axial core 321 and outer core 322 remain in constant electrical contact. Because any Mg(OH)<sub>2</sub> coating on the first metal is incomplete, electrolyte contacts both the axial and outer cores 321 and 322, respectively. In the embodiment, the part of the article made of the more reactive first metal will corrode faster, and the material of the seating portion 311 therefore does not govern the galvanic interaction.

It is noted that axial core 321 and outer core 322 remain in constant electrical contact. Because any Mg(OH)<sub>2</sub> coating on the first metal is incomplete, electrolyte contacts both the axial core 321 and the outer core 322. In this embodiment, the part of the article (e.g., the ball) made of the more active first metal will corrode faster, and the material of the seating portion 311 therefore does not affect the corrosion of the axial or outer cores 321 or 322.

FIG. 3B shows a cross-sectional view of a downhole assembly 300a similar to that of FIG. 3A but after corrosion of the first metal (where the axial core 321a comprises the first metal), with a ball 320a having a channel 321a (corresponding to the axial core 321 in FIG. 3A, now removed) surrounded by an outer core 322, and a seat 310 having a seating portion 311 made of a second metal and contained in a housing 312. The channel 321a allows only a limited opening between zones above and below the seated ball, to restrict the flow of fluid between these to an intermediate level.

In another embodiment, a frack plug of the first metal and having a ball or check valve of the first metal has a cap of an additional active material, such as a reactive magnesium alloy powder that is more reactive than the first metal, placed on top of the plug. In this way, the corrosion of the additional active material by contact with the less reactive frack plug/ball/check valve allows access to the ball or check valve.

While one or more embodiments have been shown and described, modifications and substitutions may be made thereto without departing from the spirit and scope of the invention. Accordingly, it is to be understood that the present invention has been described by way of illustrations and not limitation.

All ranges disclosed herein are inclusive of the endpoints, and the endpoints are independently combinable with each other. The suffix "(s)" as used herein is intended to include both the singular and the plural of the term that it modifies, thereby including at least one of that term (e.g., the colorant(s) includes at least one colorants). "Optional" or "optionally" means that the subsequently described event or circumstance can or cannot occur, and that the description includes instances where the event occurs and instances where it does not. As used herein, "combination" is inclusive of blends, mixtures, alloys, reaction products, and the like. All references are incorporated herein by reference.

The use of the terms "a" and "an" and "the" and similar referents in the context of describing the invention (especially in the context of the following claims) are to be construed to cover both the singular and the plural, unless otherwise indicated herein or clearly contradicted by context. Further, it should further be noted that the terms "first," "second," and the like herein do not denote any order, quantity, or importance, but rather are used to distinguish one element from another. The modifier "about" used in connection with a quantity is inclusive of the stated value and has the meaning dictated by the context (e.g., it includes the degree of error associated with measurement of the particular quantity).

The invention claimed is:

1. A method of removing a downhole assembly, comprising
  - contacting, in the presence of an electrolyte, a first article comprising a first material and acting as an anode, and
  - a second article comprising a second material having a lower reactivity than the first material and acting as a cathode,
 the downhole assembly comprising the first article in electrical contact with the second article, wherein at least a portion of the first article is corroded in the electrolyte; and
  - wherein the first material comprises a magnesium alloy having less than or equal to about 0.5 weight percent of nickel.
2. The method of claim 1, wherein the first article has a non-metallic coating on a surface thereof.
3. The method of claim 2, wherein the coating comprises a soluble glass, a soluble polymer, or a metal oxide or hydroxide coating.
4. The method of claim 2, wherein the non-metallic coating is magnesium hydroxide.
5. The method of claim 2, wherein the non-metallic coating is removed by application of an electric potential to establish electrical contact between the first and second articles.
6. The method of claim 1, wherein the second material comprises steel, tungsten, chromium, nickel, cobalt, copper, iron, aluminum, zinc, alloys thereof, or a combination comprising at least one of the foregoing.
7. The method of claim 1, wherein the first article is a controlled electrolytic material (CEM) ball or fracture plug.
8. The method of claim 1, wherein the second article is a ball seat.
9. The method of claim 1, wherein the first article comprises:
  - a corrodible core comprising the first material and at least partially penetrating the first article, and
  - a non-corrodible surrounding structure comprising the second material,
 wherein only the core is corroded.
10. The method of claim 1, wherein the first article comprises:
  - a non-corrodible core comprising the second material and at least partially penetrating the first article, and
  - a corrodible surrounding structure comprising the first material,
 wherein only the surrounding structure is corroded.
11. The method of claim 1, wherein the electrolyte is water, brine, acid, or a combination comprising at least one of the foregoing.
12. The method of claim 1, wherein the first material and the second material are selected such that the first material has a corrosion rate of about 0.1 to about 150 mg/cm<sup>2</sup>/hour using aqueous 3 wt % KCl at 200° F.
13. The method of claim 1, wherein the magnesium alloy in the first material further comprises one or more of the following: Al; Cd; Ca; Co; Cu; Fe; Mn; Si; Ag; Sr; Th; Zn; or Zr.

14. A method of producing an electrical potential in a downhole assembly, comprising
  - contacting, with an electrolyte, a first article, the first article comprising a first material and acting as an anode, and
  - a second article, the second article comprising a second material having a lower reactivity than the material of the first article and acting as a cathode,
 with a conductive element to form a circuit; wherein the first material comprises a magnesium alloy having less than or equal to about 0.5 weight percent of nickel.
15. The method of claim 14, wherein the electrolyte is water, brine, an acid, or a combination comprising at least one of the foregoing.
16. The method of claim 14, wherein the second material comprises steel, tungsten, chromium, nickel, cobalt, copper, iron, aluminum, zinc, alloys thereof, or a combination comprising at least one of the foregoing.
17. The method of claim 14, further comprising corroding the first article in the electrolyte.
18. A downhole assembly, comprising:
  - a first article comprising a first material and acting as an anode, and
  - a second article comprising a second material having a lower reactivity than the first material and acting as a cathode,
 the first and second articles being electrically connected by a conductive element to form a circuit, wherein in the presence of an electrolyte, the downhole assembly produces an electrical potential, and at least a portion of the first article is corroded; and
  - wherein the first material comprises a magnesium alloy having less than or equal to about 0.5 weight percent of nickel.
19. The article of claim 18, wherein the second material comprises steel, tungsten, chromium, nickel, cobalt, copper, iron, aluminum, zinc, alloys thereof, or a combination comprising at least one of the foregoing.
20. The article of claim 18, wherein the first article is a ball, and the second article is a ball seat.
21. A method of removing a downhole assembly, comprising:
  - contacting, in the presence of an electrolyte, a first article comprising a first material and acting as an anode, and
  - a second article comprising a second material having a lower reactivity than the first material and acting as a cathode,
 the downhole assembly comprising the first article in electrical contact with the second article, wherein at least a portion of the first article is corroded in the electrolyte; and
  - wherein the first article has a non-metallic coating comprising magnesium hydroxide on a surface thereof.

\* \* \* \* \*